



US011085152B2

(12) **United States Patent**  
**Spender et al.**

(10) **Patent No.:** **US 11,085,152 B2**  
(45) **Date of Patent:** **Aug. 10, 2021**

(54) **BIOBASED BARRIER COATINGS  
COMPRISING POLYOL/SACCHARIDE  
FATTY ACID ESTER BLENDS**

(71) Applicant: **GREENTECH GLOBAL PTE. LTD.**,  
Singapore (SG)

(72) Inventors: **Jonathan Spender**, Enfield, ME (US);  
**Michael Albert Bilodeau**, Brewer, ME  
(US); **Samuel Mikail**, Kew Gardens,  
NY (US)

(73) Assignee: **GREENTECH GLOBAL PTE. LTD.**,  
Singapore (SG)

(\*) Notice: Subject to any disclaimer, the term of this  
patent is extended or adjusted under 35  
U.S.C. 154(b) by 26 days.

(21) Appl. No.: **16/456,499**

(22) Filed: **Jun. 28, 2019**

(65) **Prior Publication Data**

US 2020/0095731 A1 Mar. 26, 2020

**Related U.S. Application Data**

(60) Provisional application No. 62/736,919, filed on Sep.  
26, 2018.

(51) **Int. Cl.**

**D21H 21/16** (2006.01)  
**D21H 19/12** (2006.01)  
**D21H 19/46** (2006.01)  
**D21H 19/52** (2006.01)  
**D21H 19/54** (2006.01)  
**D21H 19/40** (2006.01)  
**D21H 19/38** (2006.01)

(52) **U.S. Cl.**

CPC ..... **D21H 21/16** (2013.01); **D21H 19/12**  
(2013.01); **D21H 19/385** (2013.01); **D21H**

**19/40** (2013.01); **D21H 19/46** (2013.01);  
**D21H 19/52** (2013.01); **D21H 19/54** (2013.01)

(58) **Field of Classification Search**

None  
See application file for complete search history.

(56) **References Cited**

FOREIGN PATENT DOCUMENTS

WO WO 01/44420 \* 6/2001

OTHER PUBLICATIONS

“Coconut Oil, Food Data Central Search Results”, USDA Agricultural Research Service, 2020,6 pages, [online], retrieved from Internet, [retrieved Jan. 25, 2021],<URL:https://fdc.nal.usda.gov/fdc-app.html>. (Year: 2020).\*

Suryanto et al, Production of Biodiesel from Coconut Oil Using Microwave: Effect of Some Parameters on Transesterification Reaction by NaOH Catalyst, Bull Chem React Eng & Cat,v.10, No. 2,pp. 162-168,[online], retr. from Internet, [retr Jan. 25, 2021],<URL: https://doi.org/10.9767/bcrec.10.2.8080.162-168>. (Year: 2015).\*

\* cited by examiner

*Primary Examiner* — Dennis R Cordray

(74) *Attorney, Agent, or Firm* — Sughrue Mion, PLLC

(57) **ABSTRACT**

The present invention describes tunable methods of treating cellulosic materials with a barrier coating comprising at least two polyol and/or saccharide fatty acid ester that provides increased water, oil and grease resistance to such materials without sacrificing the biodegradability thereof. The methods as disclosed provide for adhering of the barrier coating on articles including articles comprising cellulosic materials and articles made by such methods. The materials thus treated display higher hydrophobicity and lipophobicity and may be used in any application where such features are desired.

**20 Claims, 7 Drawing Sheets**



FIG. 1



FIG. 2



FIG. 3



FIG. 4



FIG. 5



FIG. 6



FIG. 7

## 1

**BIOBASED BARRIER COATINGS  
COMPRISING POLYOL/SACCHARIDE  
FATTY ACID ESTER BLENDS**

**CROSS REFERENCE TO RELATED  
APPLICATIONS**

This claims benefit under 35 U.S.C. § 119(e) to U.S. Provisional Application No. 62/736,919, filed Sep. 26, 2018, which is incorporated by reference herein in its entirety.

**BACKGROUND OF THE INVENTION**

**Field of the Invention**

The present invention relates generally to treating cellulosic-compound containing materials, and more specifically to making cellulose-based materials more hydrophobic and lipophobic using biobased barrier coatings and/or compositions containing polyol and/or saccharide fatty acid ester blends, where such barrier coatings or compositions and methods are useful in modifying surfaces of cellulose-based materials including paper, paperboard and packaging products.

**Background Information**

Cellulosic materials have a wide range of applications in industry as bulking agents, absorbents, and printing components. Their employment is preferred to that of other sources of material for their high thermal stability, good oxygen barrier function, and chemical/mechanical resilience (see, e.g., Aulin et al., *Cellulose* (2010) 17:559-574; herein incorporated by reference in its entirety). Of great relevance is also the fact that these materials are fully biodegradable once dispersed in the environment, and that they are totally nontoxic. Cellulose and derivatives thereof are the material of choice for environmentally friendly solutions in applications such as packaging for foodstuff and disposable goods.

The many advantages of cellulose are nonetheless countered by the hydrophilicity/lipophilicity of the material, which shows a high affinity for water/fats and are easily hydrated (see, e.g., Aulin et al., *Langmuir* (2009) 25(13): 7675-7685; herein incorporated by reference in its entirety). While this is a benefit for applications such as absorbents and tissues, it becomes an issue when the safe packaging of watery/lipid containing materials (e.g., foodstuffs) is required. Long term storage of food, especially ready-made meals which contain a significant amount of water and/or fat, is made problematic in cellulose trays, for example, as they would first become soggy and then ultimately fail. Further, multiple coatings may be required to offset low efficiency of maintaining sufficient coating on the cellulosic surface due to the high relative porosity of the material, resulting in increased costs.

This problem is usually addressed in the industry by coating the cellulose fiber with some kind of hydrophobic organic material/fluorocarbons, silicones, which would physically shield the underlying hydrophilic cellulose from the water/lipids in the contents, including the prevention of wicking in the fiber interstices, grease flowing into creases, or allowing the release of attached materials. For example, materials such as PVC/PEI/PE are routinely used for this purpose and are physically attached (i.e., spray coated or extruded) on the surfaces to be treated.

Industry has utilized compounds based on fluorocarbon chemistry for many years to produce articles having

## 2

improved resistance to penetration by oil and grease, due to the ability of fluorocarbons to lower the surface energy of the articles. One emerging issue with the use of perfluorinated hydrocarbons is that they are remarkably persistent in the environment. The EPA and FDA have recently begun a review of the source, environmental fate, and toxicity of these compounds. A recent study reported a very high (>90%) rate of occurrence of perfluorooctane sulfonate in blood samples taken from school children. The expense and potential environmental liability of these compounds has driven manufacturers to seek alternative means of producing articles having resistance to penetration by oil and grease.

While lowering the surface energy improves the penetration resistance of the articles, lowering the surface energy also has some disadvantages. For example, a textile fabric treated with a fluorocarbon will exhibit good stain resistance; however, once soiled, the ability of cleaning compositions to penetrate and hence release the soil from the fabric may be affected, which can result in permanently soiled fabrics of reduced useful life. Another example is a grease-proof paper which is to be subsequently printed and/or coated with an adhesive. In this case the requisite grease resistance is attained by treatment with the fluorocarbon, but the low surface energy of the paper may cause problems related to printing ink or adhesive receptivity, including blocking, back trap mottle, poor adhesion, and register. If a greaseproof paper is to be used as a release paper having an adhesive applied, the low surface energy may reduce the strength of the adhesion. To improve their printability, coat-ability or adhesion, the low surface energy articles can be treated by post forming processes such as corona discharge, chemical treatment, flame treatment, or the like. However, these processes increase the cost of producing the articles and may have other disadvantages.

It would be desirable to design a "green", biobased coating which is hydrophobic, lipophobic and compostable, including a base paper/film that would allow for keeping coatings on the surface of said paper and preventing wicking into the fiber interstices, or reducing sticking of materials to the cellulosic surface, at reduced costs, without sacrificing biodegradability and/or recyclability.

**SUMMARY OF THE INVENTION**

The present disclosure relates to methods of treating cellulosic materials, including treating cellulose-containing materials with a composition that provides increased hydrophobicity and lipophobicity while maintaining biodegradability/recyclability of the cellulosic components. By using combinations of polyol or sucrose fatty acid esters (PFAE or SFAE, respectively), which fatty acid ester having, inter alia, select HLB values and degrees of substitution (DS), such combinations may be used to prepare coatings which afford water resistance, grease resistance or a combination or both to applied substrates (e.g., cellulose). The methods as disclosed include applying a barrier coating comprising a blend of PFAEs or SFAEs on cellulose.

In embodiments, a barrier coating is disclosed including at least two polyol fatty acid esters (PFAE) or saccharide fatty acid esters (SFAE), where at least one of the at least two PFAEs or SFAEs has an HLB value of equal to or less than 3 and at least one of the at least two PFAEs or SFAEs has an HLB value of equal to or greater than 7.

In one aspect, each one of the PFAEs or SFAEs possesses a different degree of substitution (DS).

In another aspect, when the coating contains a first SFAE having an HLB value of 3 and second SFAE having an HLB

value of greater than 7, the HST value of a substrate comprising the coating is greater than the combined HST values of a coating containing only the first or second SFAEs.

In one aspect, the coating is present at a sufficient concentration to cause a surface of an article containing the coating to become substantially resistant to application of water, oil and/or grease in the absence of a secondary lipophobe or hydrophobe.

In another aspect, one of the at least two SFAEs contains 1 to 5 fatty acid moieties.

In one aspect, the fatty acid moieties are saturated or are a combination of saturated and unsaturated fatty acids.

In another aspect, the coating further contains one or more compositions including clay, precipitated calcium carbonate (PCC), ground calcium carbonate (GCC), natural and/or synthetic latexes, prolamines, PvOH, TiO<sub>2</sub>, talc, glyoxal, modified starches, kaolin and combinations thereof. In a related aspect, when the coating is applied to a substrate, the coating improves the HST and 3M Kit value of said substrate compared to a coating comprising the at least two PFAEs or SFAEs alone. In a further related aspect, the coating comprises clay, GCC or PCC.

In one aspect, at least one of the two PFAEs or SFAEs is a monoester or a diester.

In another aspect, at least one PFAE or SFAE is a penta-, hexa-, hepta-, or octa-ester or a mixture thereof. In one aspect, the barrier coating is biodegradable and/or compostable. In a related aspect, the substrate includes paper, paperboard, paper pulp, a carton for food storage, fruit, a bag for food storage, a shipping bag, a container for coffee or tea, a tea bag, bacon board, diapers, weed-block/barrier fabric or film, mulching film, plant pots, packing beads, bubble wrap, oil absorbent material, laminates, envelopes, gift cards, credit cards, gloves, raincoats, OGR paper, a shopping bag, a compost bag, release paper, eating utensil, container for holding hot or cold beverages, cup, paper towels, plate, a bottle for carbonated liquid storage, insulating material, a bottle for non-carbonated liquid storage, film for wrapping food, a garbage disposal container, a food handling implement, a lid for a cup, a fabric fibre, a water storage and conveying implement, a storage and conveying implement for alcoholic or non-alcoholic drinks, an outer casing or screen for electronic goods, an internal or external piece of furniture, a curtain, upholstery, film, box, sheet, tray, pipe, water conduit, packaging for pharmaceutical products, clothing, medical device, contraceptive, camping equipment, cellulosic material that is molded and combinations thereof.

In embodiments, a method for tuneably derivatizing a cellulose-based material for lipid and water resistance is disclosed including contacting the cellulose-based material with a barrier coating comprising at least two polyol fatty acid esters (PFAE) or saccharide fatty acid esters (SFAE) and exposing the contacted cellulose-based material to heat, radiation, a catalyst or combination thereof for a sufficient time to adhere the barrier coating to the cellulose based material, where at least one of the at least two PFAEs or SFAEs has an HLB value of equal to or less than 3 and at least one of the at least two PFAEs or SFAEs has an HLB value of equal to or greater than 7.

In one aspect, the resulting cellulose-based material is substantially resistant to application of water, oil and/or grease in the absence of a secondary lipophobe or hydrophobe. In a related aspect, the resulting cellulose-based material is substantially resistant to application of water and grease.

In embodiments, a barrier coating is disclosed including at least two polyol fatty acid esters (PFAEs) or saccharide fatty acid esters (SFAEs) and one or more inorganic particles, wherein at least one of the at least two PFAEs or SFAEs has an HLB value of equal to or less than 3 and at least one of the at least two PFAEs or SFAEs has an HLB value of equal to or greater than 7.

In one aspect, when the coating is applied to a substrate, the coating improves the HST and 3M Kit value of said substrate compared to a coating comprising the at least two PFAEs or SFAEs alone. In a related aspect, the inorganic particles are selected from the group consisting of clay, talc, precipitated calcium carbonate, ground calcium carbonate, TiO<sub>2</sub> and combinations thereof. In a further related aspect, each one of the PFAEs or SFAEs possesses a different degree of substitution (DS).

#### BRIEF DESCRIPTION OF THE DRAWINGS

FIG. 1 shows a scanning electron micrograph (SEM) of untreated, medium porosity Whatman Filter Paper (58x magnification).

FIG. 2 shows an SEM of untreated, medium porosity Whatman Filter Paper (1070x magnification).

FIG. 3 shows a side-by-side comparison of SEMs of paper made from recycled pulp before (left) and after (right) coating with microfibrillated cellulose (MFC) (27x magnification).

FIG. 4 shows a side-by-side comparison of SEMs of paper made from recycled pulp before (left) and after (right) coating with MFC (98x magnification).

FIG. 5 shows water penetration in paper treated with various coating formulations: polyvinyl alcohol (PvOH), diamonds; SEFOSE®+PvOH at 1:1 (v/v), squares; Ethylex (starch), triangles; SEFOSE®+PvOH at 3:1 (v/v), crosses.

FIG. 6 shows water beading on paper treated with an aqueous composition comprising C-1803, SE-15 and precipitated calcium carbonate.

FIG. 7 Graphic illustration of HLB and ester composition.

#### DETAILED DESCRIPTION OF THE INVENTION

Before the present composition, methods, and methodologies are described, it is to be understood that this invention is not limited to particular compositions, methods, and experimental conditions described, as such compositions, methods, and conditions may vary. It is also to be understood that the terminology used herein is for purposes of describing particular embodiments only, and is not intended to be limiting, since the scope of the present invention will be limited only in the appended claims.

As used in this specification and the appended claims, the singular forms "a", "an", and "the" include plural references unless the context clearly dictates otherwise. Thus, for example, references to "a saccharide fatty acid ester" includes one or more saccharide fatty acid esters, and/or compositions of the type described herein which will become apparent to those persons skilled in the art upon reading this disclosure and so forth.

Unless defined otherwise, all technical and scientific terms used herein have the same meaning as commonly understood by one of ordinary skill in the art to which this invention belongs. Any methods and materials similar or equivalent to those described herein may be used in the practice or testing of the invention, as it will be understood

that modifications and variations are encompassed within the spirit and scope of the instant disclosure.

As used herein, "about," "approximately," "substantially" and "significantly" will be understood by a person of ordinary skill in the art and will vary in some extent depending on the context in which they are used. If there are uses of the term which are not clear to persons of ordinary skill in the art given the context in which it is used, "about" and "approximately" will mean plus or minus <10% of particular term and "substantially" and "significantly" will mean plus or minus >10% of the particular term. "Comprising" and "consisting essentially of" have their customary meaning in the art.

The present disclosure provides compositions and methods for making cellulosic surfaces both water resistant and oil/grease resistant, including producing stable aqueous barrier coatings and/or compositions for such purposes (see, e.g., FIG. 6). In the figure, the water beads were sitting on the treated paper for 1/2-hour, showing good contact angle (i.e., >90°), except for the upper right-hand portion of the sheet which was uncoated. In a related aspect, this effect requires no binder and composition-adherence to the surface is relatively permanent.

In a related aspect, the composition achieves these barrier properties while producing articles having high surface energy. As a result, the compositions avoid the disadvantages associated with the use of barrier compositions that lower the surface energy of articles. As disclosed herein, mixing saccharide/polyol fatty acid esters creates blends of such esters, which when applied as a coating to untreated papers gives both grease and water resistance. In embodiments, the ester mixtures alone, in the absence of inorganic particles or other polymers (e.g., starch or PVOH or latex), were shown to impart oil and water resistance.

In embodiments, the present disclosure shows that by 35 treating the surface of a substrate with barrier compositions comprising polyol/saccharide fatty acid ester blends the resulting surface is, *inter alia*, made resistant to water, oil and grease. The polyol/saccharide fatty acid ester blends, for example, once removed by bacterial enzymes, are easily 40 digested as such, thus the biodegradability of the substrate is not affected by the barrier coating. The barrier compositions as disclosed herein are therefore an ideal solution for derivatizing the surface of cellulose substrates to produce articles having a high surface energy.

In one aspect, where typically grease does absorb into paper, it does not readily "wick" or saturate the sheet. With a traditional barrier film a pinhole in the film becomes a conduit for all the grease on top of the film be transported to the base sheet where it absorbs and spreads. The blends of 50 the present disclosure resist absorption and spreading.

In embodiments, the PFAE/SFAE blends contain mixtures of esters containing different HLBs values, different saturated fatty acids, different degrees of substitutions (DS), different saccharide moieties, different polyol moieties, and combinations thereof. In a related aspect, the HLB value of one of the at least two PFAEs/SFAEs is greater than the other PFAE/SFAE. In a further related aspect, the HLB value of one of the PFAEs/SFAEs is 3 or lower and the other is greater than three. In another related aspect, the saturated fatty acids are from separate oil seeds, wherein the oil seed include soybeans, peanuts, rapeseeds, barley, canola, sesame seeds, cottonseeds, palm kernels, grape seeds, olives, safflowers, sunflowers, copra, corn, coconuts, linseed, hazelnuts, wheat, rice, potatoes, cassavas, legumes, camelina seeds, mustard seeds, and combinations thereof. In another related aspect, one of the PFAEs/SFAEs has a degree of

substitution of 3 or fewer and the other has a degree of substitution of 4 or greater. In another aspect, the different saccharide moieties include mono-, di-, tri-saccharides, and combinations thereof. In a related aspect, polyols may include erythritol, hydrogenated starch hydrolysates, isomalt, lactitol, maltitol, mannitol, sorbitol, xylitol, and combinations thereof.

In a related aspect, contact angles may range from 50-100 degrees depending on which ester blend is used. Under 10 conditions as disclosed herein, oil and/or water is observed to form beads instead of spreading across the treated surface using these ester blends.

Advantages of the products and methods as disclosed herein include that the coating composition is made from 15 renewable agricultural resources-polyol/saccharides and vegetable oils; is biodegradable; has a low toxicity profile and suitable for food contact; may be tuned to control the coefficient of friction of the paper/paperboard surface (i.e., does not make the paper too slippery for downstream 20 processing or end use), even at high levels of water resistance; may or may not be used with special emulsification equipment or emulsification agents; and is compatible with traditional paper recycling programs: i.e., poses no adverse impact on recycling operations, like polyethylene, polylactic acid, or wax coated papers do.

Additional advantages include, but are not limited to:

- a) ester blends are able to demonstrate significant oil penetration resistance and show oil beading up on treated surfaces (i.e., high surface energy) in the absence of secondary lipophobes;
- b) ester blends improve kit and water resistance with limited amounts of carbonate added, which allows for savings on formulations, including that the barrier coating as disclosed herein overcomes problem associated with calcium carbonate and water/grease resistance (e.g., the presence of calcium carbonate in any form usually destroys any grease resistance in paper);
- c) a formulation may be made in which all of the materials (P/SFAE, inorganic particles/pigments, such as calcium carbonate, clay and the like) in a barrier coating (except water) may provide separate functionality; and
- d) ester blends show compatibility with other oil and grease resistance technologies including PvOH, zein and latex films.

45 While not being bound by theory, oil resistance may improve with favorable high aspect ratio clays. Carbonates are unfavorably shaped and may require more esters, including that it tends to reduce oil holdout, where oil loving inorganic particles like some talcs destroy performance.

As used herein, "adhere" means to stick fast to (a surface or substance).

As used herein, "barrier coating" or "barrier composition" means a material applied to a surface (or surfaces) of a substrate that blocks or hinders the contact of unwanted elements with one or more of the applied surfaces, thus stopping the contact of said unwanted elements, such as oil or grease, with the applied surface(s) of said substrate.

As used herein, "biobased" means a material intentionally made from substances derived from living (or once-living) 55 organisms. In a related aspect, material containing at least about 50% of such substances is considered biobased.

As used herein, "bind", including grammatical variations thereof, means to cohere or cause to cohere essentially as a single mass.

60 As used herein, "cellulosic" means natural, synthetic or semisynthetic materials that can be molded or extruded into objects (e.g., bags, sheets) or films or filaments, which may

be used for making such objects or films or filaments, that is structurally and functionally similar to cellulose, e.g., coatings and adhesives (e.g., carboxymethylcellulose). In another example, cellulose, a complex carbohydrate ( $C_6H_{10}O_5$ )<sub>n</sub> that is composed of glucose units, which forms the main constituent of the cell wall in most plants, is cellulosic.

As used herein, "coating weight" is the weight of a material (wet or dry) applied to a substrate. It is expressed in pounds per specified ream or grams per square meter.

As used herein, "compostable" means these solid products are biodegradable into the soil.

As used herein, "degree of substitution" means the average number of substituent fatty acid groups attached per polyol or saccharide moiety.

As used herein, "edge wicking" means the sorption of water in a paper structure at the outside limit of said structure by one or more mechanisms including, but not limited to, capillary penetration in the pores between fibers, diffusion through fibers and bonds, and surface diffusion on the fibers. In a related aspect, the saccharide fatty acid ester containing coating as described herein prevents edge wicking in treated products. In one aspect, a similar problem exists with grease/oil entering creases that may be present in paper or paper products. Such a "grease creasing effect" may be defined as the sorption of grease in a paper structure that is created by folding, pressing or crushing said paper structure.

As used herein, "effect", including grammatical variations thereof, means to impart a particular property to a specific material.

As used herein, "hydrophobe" means a substance that does not attract water. For example, waxes, rosins, resins, saccharide fatty acid esters, diketenes, shellacs, vinyl acetates, PLA, PEI, oils, fats, lipids, other water repellent chemicals or combinations thereof are hydrophobes.

As used herein, "hydrophobicity" means the property of being water-repellent, tending to repel and not absorb water.

As used herein, "high surface energy" means an article having a surface energy of at least about 32 dynes/cm, and commonly at least about 36 dynes/cm. Less than that would be considered "low surface energy". Surface energy can be measured by any suitable method, for example by contact angle measurement and the relationship between surface energies using Young's Equation.

As used herein, "lipid resistance" or "lipophobicity" means the property of being lipid-repellent, tending to repel and not absorb lipids, grease, fats and the like. In a related aspect, the grease resistance may be measured by a "3M KIT" test or a TAPPI T559 Kit test. In another related aspect, "secondary lipophobes" would be substances that have lipid resistant properties, such as per- and polyfluoroalkyls, for example.

As used herein, "cellulose-containing material" or "cellulose-based material" means a composition which consists essentially of cellulose. For example, such material may include, but is not limited to, paper, paper sheets, paperboard, paper pulp, a carton for food storage, parchment paper, cake board, butcher paper, release paper/liner, a bag for food storage, a shopping bag, a shipping bag, bacon board, insulating material, tea bags, containers for coffee or tea, a compost bag, eating utensil, container for holding hot or cold beverages, cup, a lid, plate, a bottle for carbonated liquid storage, gift cards, a bottle for non-carbonated liquid storage, film for wrapping food, a garbage disposal container, a food handling implement, a fabric fibre (e.g., cotton or cotton blends), a water storage and conveying implement,

alcoholic or non-alcoholic drinks, an outer casing or screen for electronic goods, an internal or external piece of furniture, a curtain and upholstery.

As used herein, "release paper" means a paper sheet used to prevent a sticky surface from prematurely adhering to an adhesive or a mastic. In one aspect, the coatings as disclosed herein can be used to replace or reduce the use of silicon or other coatings to produce a material having a low surface energy. Determining the surface energy may be readily achieved by measuring contact angle (e.g., Optical Tensiometer and/or High Pressure Chamber; Dyne Testing, Staffordshire, United Kingdom) or by use of Surface Energy Test Pens or Inks (see, e.g., Dyne Testing, Staffordshire, United Kingdom).

As used herein "releasable" with reference to the SFAE means that the SFAE coating, once applied, may be removed from the cellulose-based material (e.g., removable by manipulating physical properties). As used herein "non-releasable" with reference to the SFAE means that the SFAE coating, once applied, is substantially irreversibly bound to the cellulose-based material (e.g., removable by chemical means).

As used herein, "fluffy" means an airy, solid material having the appearance of raw cotton or a Styrofoam peanut. In embodiments, the fluffy material may be made from nanocellulose fibers (e.g., MFC) cellulose nanocrystals, and/or cellulose filaments and saccharide fatty acid esters, where the resulting fibers or filaments or crystals are hydrophobic (and dispersible), and may be used in composites (e.g., concretes, plastics and the like).

As used herein, "fibers in solution" or "pulp" means a lignocellulosic fibrous material prepared by chemically or mechanically separating cellulose fibers from wood, fiber crops or waste paper. In a related aspect, where cellulose fibers are treated by the methods as disclosed herein, the cellulose fibers themselves contain bound saccharide fatty acid esters as isolated entities, and where the bound cellulose fibers have separate and distinct properties from free fibers (e.g., pulp- or cellulose fiber- or nanocellulose or microfibrillated cellulose-saccharide fatty acid ester bound material would not form hydrogen bonds between fibers as readily as unbound fibers).

As used herein, "oil contact angle" means surface wetting state by contact angle measurement of an oil droplet on the said surface. For example, water-wet if the contact angle is less than 90 (i.e., surface has a preference for water); oil-wet if the contact angle is larger than 90 (i.e., surface has a preference for oil).

As used herein, "repulpable" means to make a paper or paperboard product suitable for crushing into a soft, shapeless mass for reuse in the production of paper or paperboard.

As used herein, "stable aqueous composition" means an aqueous composition which is substantially resistant to viscosity change, coagulation, and sedimentation over at least an 8-hour period when contained in a closed vessel and stored at a temperature in a range of from about 0° C. to about 60° C. Some embodiments of the composition are stable over at least a 24-hour period, and often over at least a 6-month period.

As used herein, "tunable", including grammatical variations thereof, means to adjust or adapt a process to achieve a particular result.

As used herein, "water contact angle" means the angle measured through a liquid, where a liquid/vapor interface meets a solid surface. It quantifies the wettability of the solid surface by the liquid. The contact angle is a reflection of how strongly the liquid and solid molecules interact with each

other, relative to how strongly each interacts with its own kind. On many highly hydrophilic surfaces, water droplets will exhibit contact angles of 0° to 30°. Generally, if the water contact angle is larger than 90°, the solid surface is considered hydrophobic. Water contact angle may be readily obtained using an Optical Tensiometer (see, e.g., Dyne Testing, Staffordshire, United Kingdom).

As used herein, "water vapour permeability" means breathability or a textile's ability to transfer moisture. There are at least two different measurement methods. One, the MVTR Test (Moisture Vapour Transmission Rate) in accordance with ISO 15496, describes the water vapor permeability (WVP) of a fabric and therefore the degree of perspiration transport to the outside air. The measurements determine how many grams of moisture (water vapor) pass through a square meter of fabric in 24 hours (the higher the level, the higher the breathability).

In one aspect, TAPPI T 530 Hercules size test (i.e., size test for paper by ink resistance) may be used to determine water resistance. Ink resistance by the Hercules method is best classified as a direct measurement test for the degree of penetration. Others classify it as a rate of penetration test. There is no one best test for "measuring sizing." Test selection depends on end use and mill control needs. This method is especially suitable for use as a mill control sizing test to accurately detect changes in sizing level. It offers the sensitivity of the ink float test while providing reproducible results, shorter test times, and automatic end point determination.

Sizing, as measured by resistance to permeation through or absorption into paper of aqueous liquids, is an important characteristic of many papers. Typical of these are bag, containerboard, butcher's wrap, writing, and some printing grades.

This method may be used to monitor paper or board production for specific end uses provided acceptable correlation has been established between test values and the paper's end use performance. Due to the nature of the test and the penetrant, it will not necessarily correlate sufficiently to be applicable to all end use requirements. This method measures sizing by rate of penetration. Other methods measure sizing by surface contact, surface penetration, or absorption. Size tests are selected based on the ability to simulate the means of water contact or absorption in end use. This method can also be used to optimize size chemical usage costs.

As used herein, "oxygen permeability" means the degree to which a polymer allows the passage of a gas or fluid. Oxygen permeability (D<sub>k</sub>) of a material is a function of the diffusivity (D) (i.e., the speed at which oxygen molecules traverse the material) and the solubility (k) (or the amount of oxygen molecules absorbed, per volume, in the material). Values of oxygen permeability (D<sub>k</sub>) typically fall within the range 10-150×10<sup>-11</sup> (cm<sup>2</sup> ml O<sub>2</sub>)/(s ml mmHg). A semi-logarithmic relationship has been demonstrated between hydrogel water content and oxygen permeability (Unit: Barrer unit). The International Organization for Standardization (ISO) has specified permeability using the SI unit hectopascal (hPa) for pressure. Hence D<sub>k</sub>=10<sup>11</sup> (cm<sup>2</sup> ml O<sub>2</sub>)/(s ml hPa). The Barrer unit can be converted to hPa unit by multiplying it by the constant 0.75.

As used herein "biodegradable", including grammatical variations thereof, means capable of being broken down especially into innocuous products by the action of living things (e.g., by microorganisms).

As used herein, "recyclable", including grammatical variations thereof, means a material that is treatable or that

can be processed (with used and/or waste items) so as to make said material suitable for reuse.

As used herein, "Gurley second" or "Gurley number" is a unit describing the number of seconds required for 100 cubic centimeters (deciliter) of air to pass through 1.0 square inch of a given material at a pressure differential of 4.88 inches of water (0.176 psi) (ISO 5636-5:2003)(Porosity). In addition, for stiffness, "Gurley number" is a unit for a piece of vertically held material measuring the force required to deflect said material a given amount (1 milligram of force). Such values may be measured on a Gurley Precision Instruments' device (Troy, N.Y.).

HLB—The hydrophilic-lipophilic balance of a surfactant is a measure of the degree to which it is hydrophilic or lipophilic, determined by calculating values for the different regions of the molecule.

Griffin's method for non-ionic surfactants as described in 1954 works as follows:

$$HLB = 20 * M_h / M$$

where M<sub>h</sub> is the molecular mass of the hydrophilic portion of the molecule, and M is the molecular mass of the whole molecule, giving a result on a scale of 0 to 20. An HLB value of 0 corresponds to a completely lipophilic/hydrophobic molecule, and a value of 20 corresponds to a completely hydrophilic/lipophilic molecule.

The HLB value can be used to predict the surfactant properties of a molecule:

- <10: Lipid-soluble (water-insoluble)
- >10: Water-soluble (lipid-insoluble)
- 1.5 to 3: anti-foaming agent
- 3 to 6: W/O (water in oil) emulsifier
- 7 to 9: wetting and spreading agent
- 13 to 15: detergent
- 12 to 16: O/W (oil in water) emulsifier
- 15 to 18: solubiliser or hydrotrope

The relationship between HLB values and ester composition is shown in FIG. 7.

As may be seen in FIG. 7, in general, to have an HLB value of "1" the amount of mono-, di- and tri-ester is relatively low compared to the amount of poly esters (i.e., tetra-, penta-, hexa-, hepta-, and octaester). Further, for an HLB value of "16", the amount of monoester is relatively high compared to the amount of poly ester. Thus, by adjusting the proportion of the various esters, different HLB values may be obtained.

In some embodiments, the HLB values for the polyol or saccharide fatty acid esters (or composition comprising said ester) as disclosed herein may be in the lower range. In other embodiments, the HLB values for the saccharide fatty acid esters (or composition comprising said ester) as disclosed herein may be in the middle to higher ranges. In one aspect, the blends of P/SFAE for a stable aqueous composition entails the use of such esters where at least one of the P/SFAEs has an HLB value of 3 or lower, and another has an HLB value greater than 3.

As used herein, ISEFOSE® denotes a sucrose fatty acid ester made from soybean oil (soyate) which is commercially available from Procter & Gamble Chemicals (Cincinnati, Ohio) under the trade name SEFOSE 1618U (see sucrose polysoyate below), which contains one or more fatty acids that are unsaturated. As used herein, OLEAN® denotes a sucrose fatty acid ester which is available from Procter & Gamble Chemicals having the formula C<sub>n+12</sub>H<sub>2n+22</sub>O<sub>13</sub>, where all fatty acids are saturated.

Other SFAEs having various HLB values and variety of fatty acid moieties may be obtained from Mitsubishi Chemi-

## 11

cal Foods Corporation (Tokyo, JAPAN), under the trade-name RYOTO. Further, SFAEs may be obtained from Food-ing Group Ltd. (e.g., SE-15; Shanghai, CHINA).

As used herein, "soyate" means a mixture of salts of fatty acids from soybean oil.

As used herein, "oilseed fatty acids" means fatty acids from plants, including but not limited to soybeans, peanuts, rapeseeds, barley, canola, sesame seeds, cottonseeds, palm kernels, grape seeds, olives, safflowers, sunflowers, copra, corn, coconuts, linseed, hazelnuts, wheat, rice, potatoes, cassavas, legumes, camelina seeds, mustard seeds, and combinations thereof.

As used herein, "plasticizer" means additives that increase the plasticity or decrease the viscosity of a material. These are the substances which are added in order to alter their physical properties. These are either liquids with low volatility or maybe even solids. They decrease the attraction between polymer chains to make them more flexible.

As used herein, "polyol" means an organic compound containing multiple hydroxyl groups.

As used herein "wet strength" means the measure of how well the web of fibers holding the paper together can resist a force of rupture when the paper is wet. The wet strength may be measured using a Finch Wet Strength Device from Thwing-Albert Instrument Company (West Berlin, N.J.). Where the wet strength is typically effected by wet strength additives such as epichlorohydrin resins, including epoxide resins. In embodiments, SFAE coated cellulose based material as disclosed herein effects such wet strength in the absence of such additives.

As used herein "wet" means covered or saturated with water or another liquid.

In embodiments, a process as disclosed herein includes adhering of the barrier coating to a cellulosic surface or contacting a cellulosic surface with said barrier coating which can bind to a cellulosic surface, where said process comprises contacting a cellulose-based material with the coating comprising a polyol or saccharide fatty acid ester blend and exposing the contacted cellulose-based material to heat, radiation, a catalyst or a combination thereof for a sufficient time to bind the barrier coating to the cellulose based material. In a related aspect, such radiation may include, but is not limited to UV, IR, visible light, or a combination thereof. In another related aspect, the reaction may be carried out at room temperature (i.e., 25° C.) to about 150° C., about 50° C. to about 100° C., or about 60° C. to about 80° C.

In one aspect, the polyol or saccharide fatty acid ester blend barrier composition may contain a mixture of tri-, tetra-, or penta-esters. In another aspect, the barrier coating may contain other proteins, polysaccharides and lipids, including but not limited to, milk proteins (e.g., casein, whey protein and the like), wheat glutens, gelatins, soy protein isolates, starches, modified starches, acetylated polysaccharides, alginates, carrageenans, chitosans, inulins, long chain fatty acids, waxes, and combinations thereof.

In embodiments, the coating may additionally contain polyvinyl alcohol (PvOH).

In embodiments, no catalysts and no organic carriers (e.g., volatile organic compounds) are required to carry out adhering the coating to the article surface, including that no build-up of material is contemplated using the method as disclosed. In a related aspect, the reaction time is substantially instantaneous. Further, the resulting material exhibits low blocking.

As disclosed herein, fatty acid esters of all saccharides, including mono-, disaccharides and tri-saccharides, are

## 12

adaptable for use in connection with this aspect of the present invention. In a related aspect, the polyol/saccharide fatty acid ester may be a mono-, di-, tri-, tetra-, penta-, hexa-, hepta-, or octaester, and combinations thereof, including that the fatty acid moieties may be saturated, unsaturated or a combination thereof.

While not being bound by theory, the interaction between the polyol/saccharide fatty acid ester and the cellulose-based material may be by ionic, hydrophobic, hydrogen, van der Waals interaction, or covalent bonding, or a combination thereof. In a related aspect, the polyol/saccharide fatty acid ester binding to the cellulose-based material is substantially irreversible (e.g., using an P/SFAE comprising a combination of saturated and unsaturated fatty acids).

Further, at a sufficient concentration, the binding of the polyol or saccharide fatty acid ester alone is enough to make the cellulose-based material oil and grease resistance: i.e., lipophobicity is achieved in the absence of the addition of waxes, rosins, resins, diketenes, shellacs, vinyl acetates, natural and/or synthetic latexes, PLA, PEI, oils, other oil/grease repellent chemicals or combinations thereof (i.e., secondary lipophobes), including that other properties such as, *inter alia*, strengthening, stiffening, and bulking of the cellulose-based material may be achieved by PFAE or SFAE binding alone.

An advantage of the invention as disclosed is that multiple fatty acid chains are reactive with the cellulose, and with the two saccharide molecules in the structure, for example, the sucrose fatty acid esters as disclosed give rise to a stiff crosslinking network, leading to strength improvements in fibrous webs such as paper, paperboard, air-laid and wet-laid non-wovens, and textiles. This is typically not found in other sizing chemistries. In embodiments, a method of producing an article is disclosed using the barrier coatings above, which method produces an article which has a high surface energy and resistance to oil and grease penetration.

The invention also relates to an article which comprises the above-described composition applied to a substrate. The article has a high surface energy and resistance to water, oil and grease penetration.

Another advantage is that the polyol/saccharide fatty acid esters as disclosed soften the fibers, increasing the space between them, thus, increasing bulk without substantially increasing weight. In addition, fibers and cellulose-based material modified as disclosed herein, may be repulped. Further, for example, water, oil and grease cannot be easily "pushed" past the barrier into the sheet treated with the barrier coating as described.

Saturated PFAE and SFAE are typically solids at nominal processing temperatures, whereas unsaturated PFAE and SFAE are typically liquids. This permits the formation of uniform, stable dispersions of saturated PFAE and SFAE in aqueous coatings without significant interactions or incompatibilities with other coating components. In addition, this dispersion allows for high concentrations of saturated PFAE and SFAE to be prepared without adversely affecting coating rheology, uniform coating application, or coating performance characteristics, hence the ability to use a size press for the coatings as described herein. The coating surface will become lipophobic when the particles of comprising blends of saturated PFAE or SFAE melt and spread upon heating, drying and consolidation of the coating layer. Formed fiber products made using the method as disclosed may include paper plates, drink holders (e.g., cups), lids, food trays and packaging that would be light weight, strong, and be resistant to exposure to oil, grease, water and other liquids.

In embodiments, polyol or saccharide fatty acid esters are mixed produce sizing agents for water, oil and grease resistant coatings. As disclosed herein, the P/SFAE blends are applied to make a cellulosic surface water, oil and grease resistant in the absence of binders or secondary lipophobes or hydrophobes.

In embodiments, the saccharide fatty acid esters comprise or consist essentially of sucrose esters of fatty acids. Many methods are known and available for making or otherwise providing the saccharide fatty acid esters of the present invention, and all such methods are believed to be available for use within the broad scope of the present invention. For example, in certain embodiments it may be preferred that the fatty acid esters are synthesized by esterifying a saccharide with one or more fatty acid moieties obtained from oil seeds including but not limited to, soybean oil, sunflower oil, olive oil, canola oil, peanut oil, and mixtures thereof.

In embodiments, the saccharide fatty acid esters comprise a saccharide moiety, including but not limited to a sucrose moiety, which has been substituted by an ester moiety at one or more of its hydroxyl hydrogens. In a related aspect, disaccharide esters have the structure of Formula I.

Formula I 25



where "A" is hydrogen or of Structure I below:

Structure I



where "R" is a linear, branched, or cyclic, saturated or unsaturated, aliphatic or aromatic moiety of about eight to about 40 carbon atoms, and where at least one "A," is at least one, at least two, at least three, at least four, at least five, at least six, at least seven, and all eight "A" moieties of Formula I are in accordance with Structure I. In a related aspect, the saccharide fatty acid esters as described herein may be mono-, di-, tri-, tetra-, penta-, hexa-, hepta-, or octaesters, and combinations thereof, where the aliphatic groups may be all saturated or may contain saturated and/or unsaturated groups or combinations thereof.

Suitable "R" groups include any form of aliphatic moiety, including those which contain one or more substituents, which may occur on any carbon in the moiety. Also included are aliphatic moieties which include functional groups within the moiety, for example, an ether, ester, thio, amino, phospho, or the like. Also included are oligomer and polymer aliphatic moieties, for example sorbitan, polysorbitan and polyalcohol moieties. Examples of functional groups which may be appended to the aliphatic (or aromatic) moiety comprising the "R" group include, but are not limited to, halogens, alkoxy, hydroxy, amino, ether and ester functional groups. In one aspect, said moieties may have crosslinking functionalities. In another aspect, the SFAE may be cross-

linked to a surface (e.g., activated clay/pigment particles). In another aspect, double bonds present on the SFAE may be used to facilitate reactions onto other surfaces.

Suitable disaccharides include raffinose, maltodextrose, galactose, sucrose, combinations of glucose, combinations of fructose, maltose, lactose, combinations of mannose, combinations of erythrose, isomaltose, isomaltulose, trehalose, trehalulose, cellobiose, laminaribiose, chitobiose and combinations thereof.

10 In embodiments, the substrate for addition of fatty acids may include starches, hemicelluloses, lignins or combinations thereof.

In embodiments, a composition comprises a starch fatty acid ester, where the starch may be derived from any suitable source such as dent corn starch, waxy corn starch, potato starch, wheat starch, rice starch, sago starch, tapioca starch, sorghum starch, sweet potato starch, and mixtures thereof.

In more detail, the starch may be an unmodified starch, or a starch that has been modified by a chemical, physical, or 20 enzymatic modification.

Chemical modification includes any treatment of a starch with a chemical that results in a modified starch (e.g., plastarch material). Within chemical modification are included, but not limited to, depolymerization of a starch, oxidation of a starch, reduction of a starch, etherification of a starch, esterification of a starch, nitrification of a starch, defatting of a starch, hydrophobization of a starch, and the like. Chemically modified starches may also be prepared by using a combination of any of the chemical treatments.

30 Examples of chemically modified starches include the reaction of alkenyl succinic anhydride, particularly octenyl succinic anhydride, with starch to produce a hydrophobic esterified starch; the reaction of 2,3-epoxypropyltrimethylammonium chloride with starch to produce a cationic starch; 35 the reaction of ethylene oxide with starch to produce hydroxyethyl starch; the reaction of hypochlorite with starch to produce an oxidized starch; the reaction of an acid with starch to produce an acid depolymerized starch; defatting of a starch with a solvent such as methanol, ethanol, propanol, 40 methylene chloride, chloroform, carbon tetrachloride, and the like, to produce a defatted starch.

Physically modified starches are any starches that are physically treated in any manner to provide physically modified starches. Within physical modification are 45 included, but not limited to, thermal treatment of the starch in the presence of water, thermal treatment of the starch in the absence of water, fracturing the starch granule by any mechanical means, pressure treatment of starch to melt the starch granules, and the like. Physically modified starches 50 may also be prepared by using a combination of any of the physical treatments. Examples of physically modified starches include the thermal treatment of starch in an aqueous environment to cause the starch granules to swell without granule rupture; the thermal treatment of anhydrous starch granules to cause polymer rearrangement; fragmentation of the starch granules by mechanical disintegration; and pressure treatment of starch granules by means of an extruder to cause melting of the starch granules.

Enzymatically modified starches are any starches that are 60 enzymatically treated in any manner to provide enzymatically modified starches. Within enzymatic modification are included, but not limited to, the reaction of an alpha amylase with starch, the reaction of a protease with starch, the reaction of a lipase with starch, the reaction of a phosphorlylase with starch, the reaction of an oxidase with starch, and the like. Enzymatically modified starches may be prepared 65 by using a combination of any of the enzymatic treatments.

15

Examples of enzymatic modification of starch include the reaction of alpha-amylase enzyme with starch to produce a depolymerized starch; the reaction of alpha amylase debranching enzyme with starch to produce a debranched starch; the reaction of a protease enzyme with starch to produce a starch with reduced protein content; the reaction of a lipase enzyme with starch to produce a starch with reduced lipid content; the reaction of a phosphorylase enzyme with starch to produce an enzyme modified phosphated starch; and the reaction of an oxidase enzyme with starch to produce an enzyme oxidized starch.

Disaccharide fatty acid esters may be sucrose fatty acid esters in accordance with Formula I wherein the "R" groups

16

includes compositions which are a mixture of compounds having differing degrees of "A" group substitution, and wherein the "R" group substituent moieties are independently selected from two or more "R" groups of Structure I.

5 In a related aspect, "R" groups may be the same or may be different, including that said saccharide fatty acid esters in a composition may be the same or may be different (i.e., a mixture of different saccharide fatty acid esters).

10 For compositions of the present invention, the composition may be comprised of saccharide fatty acid ester compounds having a high degree of substitution. In embodiments, the saccharide fatty acid ester is a sucrose polysoyate.



are aliphatic and are linear or branched, saturated or unsaturated and have between about 8 and about 40 carbon atoms.

As used herein the terms "saccharide fatty acid esters" and "sucrose fatty acid ester" include compositions possessing different degrees of purity as well as mixtures of compounds of any purity level. For example, the saccharide fatty acid ester compound can be a substantially pure material, that is, it can comprise a compound having a given number of the "A" groups substituted by only one species of Structure I moiety (that is, all "R" groups are the same and all of the sucrose moieties are substituted to an equal degree). It also includes a composition comprising a blend of two or more saccharide fatty acid ester compounds, which differ in their degrees of substitution, but wherein all of the substituents have the same "R" group structure. It also

55 Saccharide fatty acid esters may be made by esterification with substantially pure fatty acids by known processes of esterification. They can be prepared also by trans-esterification using saccharide and fatty acid esters in the form of fatty acid glycerides derived, for example, from natural sources, for example, those found in oil extracted from oil seeds, for example soybean oil. Trans-esterification reactions providing sucrose fatty acid esters using fatty acid glycerides are described, for example, in U.S. Pat. Nos. 3,963,699; 4,517,360; 4,518,772; 4,611,055; 5,767,257; 6,504,003; 6,121,440; and 6,995,232, and WO1992004361 A1, herein incorporated by reference in their entireties.

60 In addition to making hydrophobic sucrose esters via transesterification, similar hydrophobic properties may be

achieved in fibrous, cellulosic articles by directly reacting acid chlorides with polyols containing analogous ring structures to sucrose.

As mentioned above, sucrose fatty acid esters may be prepared by trans-esterification of sucrose from methyl ester feedstocks which have been prepared from glycerides derived from natural sources (see, e.g., U.S. Pat. No. 6,995,232, herein incorporated by reference in its entirety). As a consequence of the source of the fatty acids, the feedstock used to prepare the sucrose fatty acid ester contains a range of saturated and unsaturated fatty acid methyl esters having fatty acid moieties containing between 12 and 40 carbon atoms. This will be reflected in the product sucrose fatty acid esters made from such a source in that the sucrose moieties comprising the product will contain a mixture of ester moiety substituents, wherein, with reference to Structure I above, the "R" groups will be a mixture having between 12 and 26 carbon atoms with a ratio that reflects the feedstock used to prepare the sucrose ester. Further to illustrate this point, sucrose esters derived from soybean oil will be a mixture of species, having "R" group structures which reflect that soybean oil comprises 26 wt. % triglycerides of oleic acid ( $\text{H}_3\text{C}-\text{CH}_2\text{}_7-\text{CH}=\text{CH}-[\text{CH}_2\text{]}_7-\text{C}(\text{O})\text{OH}$ ), 49 wt. % triglycerides of linoleic acid ( $\text{H}_3\text{C}-[\text{CH}_2\text{]}_3-[\text{CH}_2\text{}-\text{CH}=\text{CH}]\text{}_2-[\text{CH}_2\text{]}_7-\text{C}(\text{O})\text{OH}$ ), 11 wt. % of triglycerides of linolenic acid ( $\text{H}_3\text{C}-[\text{CH}_2\text{}-\text{CH}=\text{CH}]\text{}_3-[\text{CH}_2\text{]}_7-\text{C}(\text{O})\text{OH}$ ), and, 14 wt. % of triglycerides of various saturated fatty acids, as described in the Seventh Ed. Of the Merck Index, which is incorporated herein by reference. All of these fatty acid moieties are represented in the "R" groups of the substituents in the product sucrose fatty acid ester. Accordingly, when referring to a sucrose fatty acid ester herein as the product of a reaction employing a fatty acid feed stock derived from a natural source, for example, sucrose soyate, the term is intended to include all of the various constituents which are typically found as a consequence of the source from which the sucrose fatty acid ester is prepared. In a related aspect, the saccharide fatty acid esters as disclosed may exhibit low viscosity (e.g., between about 10 to 2000 centipoise at room temperature or under standard atmospheric pressure). In another aspect, the unsaturated fatty acids, may have one, two, three or more double bonds.

In embodiments of the present invention, the polyol or saccharide fatty acid ester, and in aspects, the disaccharide ester, is formed from fatty acids having greater than about 6 carbon atoms, from about 8 to 16 carbon atoms, from about 8 to about 18 carbon atoms, from about 14 to about 18 carbons atoms, from about 16 to about 18 carbon atoms, from about 16 to about 20 carbon atoms, and from about 20 to about 40 carbon atoms, on average.

In embodiments, the ratios for polyol or saccharide fatty acid ester having different DS or HLB values in the barrier coatings, for example, may be different to achieve hydrophobicity/lipophobicity depending on the form of the cellulose-based material. In one aspect, the PFAE/SFAE ratio may be 1:1, 2:1, 3:1, 4:1 or 5:1 on a weight to weight (wt/wt) basis. In a related aspect, when different polyol or saccharide fatty acid esters (PFAE or SFAE) are mixed as a coating on the cellulose-based material, the coating weight of at least about 0.1 g/m<sup>2</sup> to about 1.0 g/m<sup>2</sup>, about 1.0 g/m<sup>2</sup> to about 2.0 g/m<sup>2</sup>, about 2 g/m<sup>2</sup> to about 3 g/m<sup>2</sup> on a surface of the cellulose-based material, may be used. In a related aspect, it may be present from about 3 g/m<sup>2</sup> to about 4 g/m<sup>2</sup>, about 4 g/m<sup>2</sup> to about 5 g/m<sup>2</sup>, about 5 g/m<sup>2</sup> to about 10 g/m<sup>2</sup>, about 10 g/m<sup>2</sup> to about 20 g/m<sup>2</sup>. In another aspect, when the cellulose-based material is a solution containing cellulose

fiber, the coating may be present at a concentration of at least about 0.025% (wt/wt) of the total fiber present. In a related aspect, it may be present at about 0.05% (wt/wt) to about 0.1% (wt/wt), about 0.1% (wt/wt) to about 0.5% (wt/wt), about 0.5% (wt/wt) to about 1.0% (wt/wt), about 1.0% (wt/wt) to about 2.0% (wt/wt), about 2.0% (wt/wt) to about 3.0% (wt/wt), about 3.0% (wt/wt) to about 4.0% (wt/wt), about 4.0% (wt/wt) to about 5.0% (wt/wt), about 5.0% (wt/wt) to about 10% (wt/wt), about 10% (wt/wt) to about 50% (wt/wt) of the total fiber present.

In other embodiments, a coating may comprise between about 0.9% to about 1.0%, about 1.0% to about 5.0%, about 5.0 to about 10%, about 10% to about 20%, about 20% to about 30%, about 30% to about 50% or greater polyol or saccharide fatty acid ester by weight of the coating (wt/wt). In a related aspect, the coating may contain between about 25% to about 35% polyol or saccharide fatty acid ester by weight of the coating (wt/wt).

In embodiments, the cellulose-based material includes, but is not limited to, paper, paperboard, paper sheets, paper pulp, cups, boxes, trays, lids, release papers/liners, compost bags, shopping bags, shipping bags, bacon board, tea bags, insulating material, containers for coffee or tea, pipes and water conduits, food grade disposable cutlery, plates and bottles, screens for TV and mobile devices, clothing (e.g., cotton or cotton blends), bandages, pressure sensitive labels, pressure sensitive tape, feminine products, and medical devices to be used on the body or inside it such as contraceptives, drug delivery devices, container for pharmaceutical materials (e.g., pills, tablets, suppositories, gels, etc.), and the like. Also, the coating technology as disclosed may be used on furniture and upholstery, outdoors camping equipment and the like.

In one aspect, the coatings as described herein are resistant to pH in the range of between about 3 to about 9. In a related aspect, the pH may be from about 3 to about 4, about 4 to about 5, about 5 to about 7, about 7 to about 9.

In embodiments, a method for treating a surface of a cellulose containing (or cellulosic) material is disclosed including applying to the surface a composition containing an alcanoic acid derivative having the formula (II) or (III):



where R is a straight-chain, branched-chain, or cyclic aliphatic hydrocarbon radical having from 6 to 50 carbon atoms, and where X and X<sub>1</sub> are independently Cl, Br, R-CO-O-R, or O(CO)OR, where when the alcanoic acid derivative comprises formula (III) X or X<sub>1</sub> is the same or is different, where the SFAE as disclosed herein is a carrier, and where the method does not require an organic base, gaseous HCl, VOCs or catalyst.

In embodiments, an alcanoic acid derivative is mixed with a saccharide fatty acid ester to form an emulsion, where the emulsion is used to treat the cellulose-based material.

In embodiments, the polyol or saccharide fatty acid ester may be an emulsifying agent and may comprise a mixture of one or more mono-, di-, tri-, tetra-, penta-, hexa-, hepta-, or octaesters, and combinations thereof. In one aspect, the polyol or saccharide fatty acid ester may be an emulsifying agent and may comprise a mixture of one or more tri-, tetra-, or penta-esters. In another aspect, the fatty acid moiety of the polyol or saccharide fatty acid ester may contain saturated groups, unsaturated groups or a combination thereof. In one aspect, the polyol or saccharide fatty acid ester-containing emulsion may contain other proteins, polysaccharides and/or

lipids, including but not limited to, milk proteins (e.g., casein, whey protein and the like), gelatins, soy protein isolates, starches, acetylated polysaccharides, alginates, carrageenans, chitosans, inulins, long chain fatty acids, waxes, and combinations thereof.

In embodiments the polyol or saccharide fatty acid ester emulsifiers as disclosed herein may be used to carry coatings or other chemicals used for paper manufacturing including, but not limited to, agalite, esters, diesters, ethers, ketones, amides, nitriles, aromatics (e.g., xylenes, toluenes), acid halides, anhydrides, talc, alkyl ketene dimer (AKD), alabaster, algenic acid, alum, albarine, glues, barium carbonate, barium sulfate, precipitated calcium carbonate, ground calcium carbonate, titanium dioxide, clays, dolomite, diethylene triamine penta acetate, EDTA, enzymes, formamidine sulfuric acid, guar gum, gypsum, lime, magnesium bisulfate, milk of lime, milk of magnesia, polyvinyl alcohol (PvOH), rosins, rosin soaps, satins, soaps/fatty acids, sodium bisulfate, soda-ash, titania, surfactants, starches, modified starches, hydrocarbon resins, polymers, waxes, polysaccharides, proteins, dyestuffs, optical brightening agents, and combinations thereof.

In embodiments, the cellulose-containing material generated by the methods as disclosed herein exhibits greater hydrophobicity and water-resistance relative to the cellulose-containing material without the treatment. In a related aspect, the treated cellulose-containing material exhibits greater lipophobicity or grease resistance relative to the cellulose-containing material without the treatment. In a further related aspect, the treated cellulose-containing material may be biodegradable, compostable, and/or recyclable.

In embodiments, the treated cellulose-containing material may have improved mechanical properties compared to that same material untreated. For example, paper bags treated by the process as disclosed herein show increased burst strength, Gurley Number, Tensile Strength and/or Energy of Maximum Load. In one aspect, the burst strength is increased by a factor of between about 0.5 to 1.0 fold, between about 1.0 and 1.1 fold, between about 1.1 and 1.3 fold, between about 1.3 to 1.5 fold. In another aspect, the Gurley Number increased by a factor of between about 3 to 4 fold, between about 4 to 5 fold, between about 5 to 6 fold and about 6 to 7 fold. In still another aspect, the Tensile Strain increased by a factor of between about 0.5 to 1.0 fold, between about 1.0 to 1.1 fold, between about 1.1 to 1.2 fold and between about 1.2 to 1.3 fold. And in another aspect, the Energy of Max Load increased by a factor of between about 1.0 to 1.1 fold, between about 1.1 to 1.2 fold, between about 1.2 to 1.3 fold, and between about 1.3 to 1.4 fold.

In embodiments, the cellulose-containing material is a base paper comprising microfibrillated cellulose (MFC) or cellulose nanofiber (CNF) as described for example in U.S. Pub. No. 2015/0167243 (herein incorporated by reference in its entirety), where the MFC or CNF is added during the forming process and paper making process and/or added as a coating or a secondary layer to a prior forming layer to decrease the porosity of said base paper. In a related aspect, the base paper is contacted with the saccharide fatty acid ester as described above. In a further related aspect, the contacted base paper is further contacted with a polyvinyl alcohol (PvOH). In embodiments, the resulting contacted base paper is tuneably water and lipid resistant. In a related aspect, the resulting base paper may exhibit a Gurley value of at least about 10-15 (i.e., Gurley Air Resistance (sec/100 cc, 20 oz. cyl.)), or at least about 100, at least about 200 to about 350. In one aspect, the polyol/saccharide fatty acid ester blend may be a laminate for one or more layers or may

provide one or more layers as a laminate or may reduce the amount of coating of one or more layers to achieve the same performance effect (e.g., water resistance, grease resistance, and the like). In a related aspect, the laminate may comprise a biodegradable and/or compostable heat seal or adhesive.

In embodiments, the polyol or saccharide fatty acid esters may be formulated as emulsions, where the choice emulsifying agent and the amount employed is dictated by the nature of the composition and the ability of the agent to 10 facilitate the dispersion of the saccharide fatty acid ester. In one aspect, the emulsifying agents may include, but are not limited to, water, buffers, polyvinyl alcohol (PvOH), carboxymethyl cellulose (CMC), milk proteins, wheat glutens, gelatins, soy protein isolates, starches, acetylated polysaccharides, alginates, carrageenans, chitosans, inulins, long 15 chain fatty acids, waxes, agar, alginates, glycerol, gums, lecithins, poloxamers, mono-, di-glycerols, monosodium phosphates, monostearate, propylene glycols, detergents, cetyl alcohol, and combinations thereof. In another aspect, 20 the saccharide ester:emulsifying agent ratios may be from about 0.1:99.9, from about 1:99, from about 10:90, from about 20:80, from about 35:65, from about 40:60, and from about 50:50. It will be apparent to one of skill in the art that ratios may be varied depending on the property(ies) desired 25 for the final product.

In embodiments, the polyol/saccharide fatty acid ester blends may be combined with one or more components for internal and surface sizing (alone or in combination), including but not limited to, pigments (e.g., clay, calcium carbonate, titanium dioxide, plastic pigment), binders (e.g., starch, soy protein, polymer emulsions, PvOH), and additives (e.g., glyoxal, glyoxalated resins, zirconium salts, calcium stearate, calcium carbonates, lecithin oleate, polyethylene emulsion, carboxymethyl cellulose, acrylic polymers, alginates, 30 polyacrylate gums, polyacrylates, microbiocides, oil based defoamers, silicone based defoamers, stilbenes, direct dyes and acid dyes). In a related aspect, such components may provide one or more properties, including but not limited to, 35 building a fine porous structure, providing light scattering surface, improving ink receptivity, improving gloss, binding pigment particles, binding coatings to paper, base sheet reinforcement, filling pores in pigment structure, reducing water sensitivity, resisting wet pick in offset printing, preventing blade scratching, improving gloss in supercalendering, 40 reducing dusting, adjusting coating viscosity, providing water holding, dispersing pigments, maintaining coating dispersion, preventing spoilage of coating/coating color, controlling foaming, reducing entrained air and coating craters, increasing whiteness and brightness, and controlling 45 color and shade. It will be apparent to one of skill in the art that combinations may be varied depending on the property(ies) desired for the final product.

In embodiments, the methods employing said polyol/saccharide fatty acid ester blends may be used to lower the 50 cost of applications of primary/secondary coating (e.g., silicone-based layer, starch-based layer, clay-based layer, PLA-layer, PEI-layer and the like) by providing a layer of material that exhibits a necessary property (e.g., oil and grease resistance, water resistance, low surface energy, high 55 surface energy, and the like), thereby reducing the amount of primary/secondary layer necessary to achieve that same property. In one aspect, materials may be coated on top of a P/SFAE layer (e.g., heat sealable agents). In embodiments, the composition is fluorocarbon and silicone free.

In embodiments, the compositions increase both mechanical and thermal stability of the treated product. In one aspect, the surface treatment is thermostable at temperatures

between about -100° C. to about 300° C. In further related aspect, the surface of the cellulose-based material exhibits a water contact angle of between about 60° to about 120°. In another related aspect, the surface treatment is chemically stable at temperatures of between about 200° C. to about 300° C.

The substrate which may be dried prior to application (e.g., at about 80-150° C.), may be treated with the modifying composition by dipping, for example, and allowing the surface to be exposed to the composition for less than 1 second. The substrate may be heated to dry the surface, after which the modified material is ready for use. In one aspect, according to the method as disclosed herein the substrate may be treated by any suitable coating/sizing process typically carried out in a paper mill (see, e.g., Smook, G., *Surface Treatments in Handbook for Pulp & Paper Technologists*, (2016), 4<sup>th</sup> Ed., Cpt. 18, pp. 293-309, TAPPI Press, Peachtree Corners, Ga. USA, herein incorporated by reference in its entirety).

No special preparation of the material is necessary in practicing this invention, although for some applications, the material may be dried before treatment. In embodiments, the methods as disclosed may be used on any cellulose-based surface, including but not limited to, a film, a rigid container, fibers, pulp, a fabric or the like. In one aspect, the polyol or saccharide fatty acid esters or coating agents may be applied by conventional size press (vertical, inclined, horizontal), gate roll size press, metering size press, calender size application, tube sizing, on-machine, off-machine, single-sided coater, double-sided coater, short dwell, simultaneous two-side coater, blade or rod coater, gravure coater, gravure printing, flexographic printing, ink-jet printing, laser printing, supercalendering, and combinations thereof.

Depending on the source, the cellulose may be paper, paperboard, pulp, softwood fiber, hardwood fiber, or combinations thereof, nanocellulose, cellulose nanofibres, whiskers or microfibril, microfibrillated, cotton or cotton blends, cellulose nanocrystals, or nanofibrillated cellulose.

In embodiments, the amount of polyol/saccharide fatty acid ester blend applied is sufficient to completely cover at least one surface of a cellulose-containing material. For example, in embodiments, the polyol/saccharide fatty acid ester blend may be applied to the complete outer surface of a container, the complete inner surface of a container, or a combination thereof, or one or both sides of a base paper. In other embodiments, the complete upper surface of a film may be covered by the polyol/saccharide fatty acid ester blend, or the complete under surface of a film may be covered by the polyol/saccharide fatty acid ester blend, or a combination thereof. In some embodiments, the lumen of a device/instrument may be covered by the coating or the outer surface of the device/instrument may be covered by the polyol/saccharide fatty acid ester blend, or a combination thereof. In embodiment, the amount of polyol/saccharide fatty acid ester blend applied is sufficient to partially cover at least one surface of a cellulose-containing material. For example, only those surfaces exposed to the ambient atmosphere are covered by the polyol/saccharide fatty acid ester blend, or only those surfaces that are not exposed to the ambient atmosphere are covered by the polyol/saccharide fatty acid ester blend (e.g., masking). As will be apparent to one of skill in the art, the amount of polyol/saccharide fatty acid ester blend applied may be dependent on the use of the material to be covered. In one aspect, one surface may be coated with a polyol/saccharide fatty acid ester blend and the opposing surface may be coated with an agent including, but not limited to, proteins, wheat glutens, gelatins, soy protein

isolates, starches, modified starches, acetylated polysaccharides, alginates, carrageenans, chitosans, inulins, long chain fatty acids, waxes, and combinations thereof. In a related aspect, the P/SFAE blend can be added to a furnish, and the resulting material on the web may be provided with an additional coating of P/SFAE or P/SFAE blend.

Any suitable coating process may be used to deliver any of the various polyol/saccharide fatty acid ester blend and/or emulsions applied in the course of practicing this aspect of the method. In embodiments, polyol/saccharide fatty acid ester blend process includes immersion, spraying, painting, printing, and any combination of any of these processes, alone or with other coating processes adapted for practicing the methods as disclosed.

It will be apparent to one of skill in the art that the selection of cellulose to be treated, the polyol/saccharide fatty acid ester blend, the reaction temperature, and the exposure time are process parameters that may be optimized by routine experimentation to suit any particular application for the final product.

The derivatized materials have altered physical properties which may be defined and measured using appropriate tests known in the art. For hydrophobicity the analytical protocol may include, but is not limited to, the contact angle measurement and moisture pick-up. Other properties include, stiffness, WVTR, porosity, tensile strength, lack of substrate degradation, burst and tear properties. A specific standardized protocol to follow is defined by the American Society for Testing and Materials (protocol ASTM D7334-08).

The permeability of a surface to various gases such as water vapour and oxygen may also be altered by the saccharide fatty acid ester coating process as the barrier function of the material is enhanced. The standard unit measuring permeability is the Barrer and protocols to measure these parameters are also available in the public domain (ASTM std F2476-05 for water vapour and ASTM std F2622-8 for oxygen).

In embodiments, materials treated according to the presently disclosed procedure display a complete biodegradability as measured by the degradation in the environment under microorganismal attack.

Various methods are available to define and test biodegradability including the shake-flask method (ASTM E1279-89(2008)) and the Zahn-Wellens test (OECD TG 302 B).

Various methods are available to define and test compatibility including, but not limited to, ASTM D6400.

In embodiments, the barrier composition as disclosed herein, when applied to a substrate, produces an article having resistance to oil and grease and water penetration. Resistance to oil and grease penetration includes resistance to penetration by various oils, greases, waxes, other oily substances and surprisingly highly penetrating solvents like toluene and heptane. The resistance to oil and grease penetration may be measured by the 3M Kit Test. In one aspect, the composition has a Kit number of at least 3, more preferably at least 5, more preferably at least 7, and most preferably at least 9.

In embodiments, methods of producing an article are disclosed comprises applying the barrier composition to a substrate to produce the article which has a high surface energy and resistance to oil and grease penetration. In a related aspect, the barrier composition is provided in intimate contact with one or more surfaces of the substrate in order to provide penetration resistance to those surfaces. In a related aspect, the barrier coating may be applied as a coating on the one or more surfaces, or in some applications

it may be applied such that it is absorbed into the interior of substrate and contacts one or more surfaces.

In embodiments, the barrier composition is applied as a coating on the substrate. The substrate may be coated with the composition by any suitable method, for example, by rolling, spreading, spraying, brushing, or pouring processes, followed by drying, by co-extruding the barrier composition with other materials onto a preformed substrate, or by melt/extrusion coating a preformed substrate. In one aspect, the coating may be applied by a size press. In another aspect, the substrate may be coated on one side or on both or all sides with the barrier composition. In another aspect, a coating knife, such as a "doctor blade", allows uniform spreading of the barrier composition onto a substrate that is moved along by rollers, may be used. In a related aspect, the barrier coating may be applied to textiles, non-wovens, foil, paper, paperboard, and other sheet materials by continuously operating spread-coating machines.

The barrier compositions as disclosed herein may be used to produce a wide variety of different articles having resistance to oil and grease penetration. The articles may include, but are not limited to, paper, paperboard, cardboard, containerboard, gypsum board, wood, wood composites, furniture, masonry, leather, automobile finishes, furniture polishes, plastics, non-stick cookware, and foams.

In embodiments, the barrier compositions as disclosed herein may be used in food packaging papers and paperboard, including fast food packaging. Specific examples of food packaging uses include fast food wrappers, food bags, snack bags, grocery bags, cups, trays, cartons, boxes, bottles, crates, food packaging films, blister pack wrappers, microwavable popcorn bags, release papers, pet food containers, beverage containers, OGR papers, and the like. In embodiments, textile articles may be produced, such as natural textile fibers or synthetic textile fibers. In a related aspect, the textile fibers may be further processed into garments, linens, carpets, draperies, wall-coverings, upholstery and the like.

In embodiments, substrates may be formed into articles prior to or after applying the barrier composition. In one aspect, containers may be produced from flat, coated paperboard by press-forming, by vacuum forming, or by folding and adhering them into the final desired shape. Coated, flat paperboard stock may be formed into trays by the application of heat and pressure, as disclosed within, for example, U.S. Pat. No. 4,900,594 (incorporated herein by reference), or vacuum formed into containers for foods and beverages, as disclosed within U.S. Pat. No. 5,294,483 (incorporated herein by reference).

Materials suitable for treatment by the process of this invention include various forms of cellulose, such as cotton fibers, plant fibers such as flax, wood fibers, regenerated cellulose (rayon and cellophane), partially alkylated cellulose (cellulose ethers), partially esterified cellulose (acetate rayon), and other modified cellulose materials which have a substantial portion of their surfaces available for reaction/binding. As stated above, the term "cellulose" includes all of these materials and others of similar polysaccharide structure and having similar properties. Among these the relatively novel material microfibrillated cellulose (cellulose nanofiber) (see e.g., U.S. Pat. No. 4,374,702 and US Pub. Nos. 2015/0167243 and 2009/0221812, herein incorporated by reference in their entireties) is particularly suitable for this application. In other embodiments, celluloses may include but are not limited to, cellulose triacetate, cellulose propionate, cellulose acetate propionate, cellulose acetate butyrate, nitrocellulose (cellulose nitrate), cellulose sulfate,

celluloid, methylcellulose, ethylcellulose, ethyl methyl cellulose, hydroxyethyl cellulose, hydroxypropyl cellulose, cellulose nanocrystals, hydroxyethyl methyl cellulose, hydroxypropyl methyl cellulose, ethyl hydroxyethyl cellulose, carboxymethyl cellulose, and combinations thereof.

The modification of the cellulose with the barrier coating as disclosed herein, in addition to increasing its resistance to oil and grease, may also increase its tensile strength, flexibility and stiffness, thereby further widening its spectrum of use. All biodegradable and partially biodegradable products made from or by using the modified cellulose disclosed in this application are within the scope of the disclosure, including recyclable and compostable products.

Among the possible applications of the coating technology such items include, but are not limited to, containers for all purpose such as paper, paperboard, paper pulp, cups, lids, boxes, trays, release papers/liners, compost bags, shopping bags, pipes and water conduits, food grade disposable cutlery, plates and bottles, screens for TV and mobile devices, clothing (e.g., cotton or cotton blends), bandages, pressure sensitive labels, pressure sensitive tape, feminine products, and medical devices to be used on the body or inside it such as contraceptives, drug delivery devices, and the like. Also, the coating technology as disclosed may be used on furniture and upholstery, outdoors camping equipment and the like.

The following examples are intended to illustrate but not limit the invention.

## EXAMPLES

### Example 1. Saccharide Fatty Acid Ester Formulations

SEFOSE® is a liquid at room temperature and all coatings/emulsions containing this material were applied at room temperature using a bench top drawdown device. Rod type and size were varied to create a range of coat weights. Formulation 1

50 ml of SEFOSE® were added to a solution containing 195 ml of water and 5 grams of carboxymethylcellulose (FINNFINX® 10; CP Kelco, Atlanta, Ga.). This formulation was mixed using a Silverson Homogenizer set to 5000 rpm for 1 minute. This emulsion was coated on a 50 gram base sheet made of bleached hardwood pulp and an 80 gram sheet composed of unbleached softwood. Both papers were placed into an oven (105° C.) for 15 minutes to dry. Upon removal from the oven, sheets were placed on the lab bench and 10 drops of water (room temperature) applied via pipette to each sheet. The base sheets selected for this testing would absorb a droplet of water immediately, whereas sheets coated with varying amounts of SEFOSE® showed increasing levels of water resistance as coat weight increased (see Table 1).

TABLE 1

| Base Sheet Results with SEFOSE® |                                            |                                      |  |
|---------------------------------|--------------------------------------------|--------------------------------------|--|
| Coat weight g/m <sup>2</sup>    | 50 g Hardwood Base Water Holdout (minutes) | 80 g Softwood Base Holdout (minutes) |  |
| 3.2                             | 1                                          | 0.5                                  |  |
| 4.1                             | 14                                         | 9                                    |  |
| 6.4                             | 30                                         | 25                                   |  |
| 8.5                             | 50                                         | 40                                   |  |
| 9.2                             | 100+                                       | 100+                                 |  |

It was observed that water resistance was less in the heavier sheet and no water resistance was achieved unless the sheet was dry.

Formulation 2

Addition of SEFOSE® to cup stock: (note this is single layer stock with no MFC treatment. 110 gram board made of Eucalyptus pulp). 50 grams of SEFOSE® was added to 200 grams of 5% cooked ethylated starch (Ethylex 2025) and stirred using a bench top kady mill for 30 seconds. Paper samples were coated and placed in the oven at 105° C. for 15 minutes. 10-15 test droplets were placed on the coated side of the board and water holdout time was measured and recorded in the table below. Water penetration on the untreated board control was instant (see Table 2).

TABLE 2

| Penetration of Hot Water for SEFOSE® Treated Cup Stock |                                      |                       |
|--------------------------------------------------------|--------------------------------------|-----------------------|
| Quantity Applied<br>g/m <sup>2</sup>                   | Time<br>Required for<br>Hot (80° C.) | Water to<br>Penetrate |
| 2.3                                                    | 0.05 hr                              |                       |
| 4.1                                                    | 0.5 hr                               |                       |
| 6.2                                                    | 1.2 hr                               |                       |
| 8.3                                                    | 3.5 hr                               |                       |
| 9.6                                                    | ~16 hr                               |                       |

Formulation 3

Pure SEFOSE® was warmed to 45° C. and placed in a spray bottle. A uniform spray was applied to the paper stock listed in the previous example, as well as to a piece of fiberboard and an amount of cotton cloth. When water drops were placed on the samples, penetration into the substrate occurred within 30 seconds, however after drying in the oven for 15 minutes at 105° C. beads of water evaporated before being absorbed into the substrate.

Continued investigation concerned whether SEFOSE® might be compatible with compounds used for oil and grease resistant coatings. SEFOSE® is useful for water resistance as well as stiffness improvements. 240 gram board stock was used to do stiffness tests. Table 3 shows the results. These data were obtained at a single coat weight: 5 grams/square meter with a 5 sample average being reported. Results are in Taber stiffness units recorded with our V-5 Taber stiffness tester Model 150-E.

TABLE 3

| Stiffness Test             |                                   |                              |
|----------------------------|-----------------------------------|------------------------------|
| Sample tested              | Machine<br>Direction<br>Stiffness | Cross Direction<br>Stiffness |
| Control board - no coating | 77.6                              | 51.8                         |
| SEFOSE®                    | 85.9                              | 57.6                         |
| Erucic Acid                | 57.9                              | 47.4                         |
| Palmitoyl chloride         | 47.7                              | 39.5                         |

Example 2. Bonding of Saccharide Ester to Cellulosic Substrate

In an effort to determine whether SEFOSE® was reversibly bound to a cellulosic material, pure SEFOSE® was mixed with pure cellulose at ratio of 50:50. The SEFOSE® was allowed to react for 15 min at 300° F. and the mixture

was extracted with methylene chloride (non-polar solvent) or distilled water. The samples were refluxed for 6 hours, and gravimetric analysis of the samples was carried out.

TABLE 4

| Extraction of SEFOSE® from Cellulosic Material |            |              |                   |                    |
|------------------------------------------------|------------|--------------|-------------------|--------------------|
| Sample                                         | Total Mass | SEFOSE® Mass | SEFOSE® Extracted | % SEFOSE® Retained |
| CH <sub>2</sub> Cl <sub>2</sub>                | 2.85       | 1.42         | 0.25              | 83%                |
| H <sub>2</sub> O                               | 2.28       | 1.14         | 0.08              | 93%                |

Example 3. Examination of Cellulosic Surfaces

Scanning electron microscope images of base papers with and without MFC illustrate how a less porous base has potential to require far less waterproofing agents reacted to the surface. FIGS. 1-2 show untreated, medium porosity Whatman filter paper. FIGS. 1 and 2 show the relative high surface area exposed for a derivitizing agent to react with; however, it also shows a highly porous sheet with plenty of room for water to escape. FIGS. 3 and 4 show a side by side comparison of paper made with recycled pulp before and after coating with MFC. (They are two magnifications of the same samples, no MCF obviously on the left side of image). The testing shows that derivitization of a much less porous sheet shows more promise for long term water/vapor barrier performance. The last two images are just close ups taken of an average “pore” in a sheet of filter paper as well as a similar magnification of CNF coated paper for contrast purposes.

The data above demonstrate a critical point: that addition of more material results in a corresponding increase in performance. While not being bound by theory, the reaction appears to be faster with unbleached papers, suggesting that the presence of lignin may speed the reaction.

The fact that a product like the SEFOSE® is a liquid, it can readily emulsify, suggesting that it can easily be adapted to work in coating equipment commonly used in paper mills.

Example 4. “Phluphi”

Liquid SEFOSE® was mixed and reacted with bleached hardwood fiber to generate a variety of ways to create a waterproof handsheet. When the sucrose ester was mixed with pulp prior to sheet formation it was found that the majority of it is retained with the fiber. With sufficient heating and drying, a brittle, fluffy but very hydrophobic handsheet was formed. In this example, 0.25 grams SEFOSE® was mixed with 4.0 grams bleached hardwood fiber in 6 Liters of water. This mixture was stirred by hand and the water drained in a standard handsheet mold. The resulting fiber mat was removed and dried for 15 minutes at 325° F. The produced sheet exhibited significant hydrophobicity as well as greatly reduced hydrogen bonding between the fibers themselves. (Water contact angle was observed to be greater than 100 degrees). An emulsifier may be added. SEFOSE® to fiber may be from about 1:100 to 2:1.

Subsequent testing shows that talc is only a spectator in this and was left out of additional testing.

Example 5. Environmental Effects on SEFOSE® Coating Properties

In an effort to better understand the mechanism of sucrose esters reaction with fiber, low viscosity coatings were

applied to a bleach kraft sheet that had wet strength resin added, but no water resistance (no sizing). Coatings were all less than 250 cps as measured using a Brookfield Viscometer at 100 rpm.

SEFOSE® was emulsified with Ethylex 2025 (starch) and applied to the paper via a gravure roll. For comparison, SEFOSE® was also emulsified with Westcote 9050 PVOH. As shown in FIG. 5, oxidation of the double bonds in SEFOSE® is enhanced by the presence of heat and additional chemical environments that enhance oxidative chemistry (see also, Table 5).

TABLE 5

| Environmental Effects on SEFOSE® (Minutes to Failure) |       |              |         |     |
|-------------------------------------------------------|-------|--------------|---------|-----|
| Time                                                  | PVOH  | SEFOSE®-PVOH | Ethylex | 3:1 |
| 0                                                     | 0.08  | 0.07         | 0.15    | 2   |
| 1                                                     | 0.083 | 0.11         | 0.15    | 1.8 |
| 2                                                     | 0.08  | 0.18         | 0.13    | 1.8 |
| 5                                                     | 0.09  | 0.25         | 0.1     | 1.3 |
| 10                                                    | 0.08  | 0.4          | 0.1     | 0.9 |
| 30                                                    | 0.08  | 1.1          | 0.08    | 0.8 |
| 60                                                    | 0.08  | 3.8          | 0.08    | 0.8 |
| 120                                                   | 0.08  | 8            | 0.08    | 0.7 |
| 500                                                   | 0.07  | 17           | 0.07    | 0.4 |

Example 6. Effect of Unsaturated vs. Saturated Fatty Acid Chains

SEFOSE® was reacted with bleached softwood pulp and dried to form a sheet. Subsequently, extractions were carried out with  $\text{CH}_2\text{Cl}_2$ , toluene and water to determine the extent of the reaction with pulp. Extractions were performed for at least 6 hours using Soxhlet extraction glassware. Results of the extractions are shown in Table 6.

TABLE 6

| Extraction of SEFOSE®-bound Pulp |         |                          |         |
|----------------------------------|---------|--------------------------|---------|
|                                  | Water   | $\text{CH}_2\text{Cl}_2$ | Toluene |
| Mass of Dry Pulp                 | 8.772 g | 9.237 g                  | 8.090 g |
| SEFOSE® added                    | 0.85 g  | 0.965 g                  | 0.798 g |
| Amount Extracted                 | 0.007 g | 0.015 g                  | 0.020 g |

The data indicate that essentially all of the SEFOSE® remains in the sheet. To further verify this, the same procedure was carried out on the pulp alone, and results show that approximately 0.01 g per 10 g of pulp was obtained. While not being bound by theory, this could easily be accounted for as residual pulping chemicals or more likely extractives that had not been completely removed.

Pure fibers of cellulose (e.g.,  $\alpha$ -cellulose from Sigma Aldrich, St. Louis, Mo.) were used, and the experiment repeated. As long as the loading levels of SEFOSE® remained below about 20% of the mass of the fibers, over 95% of the mass of SEFOSE® was retained with the fibers and not extractable with either polar or non-polar solvents. While not being bound by theory, optimizing baking time and temperature may further enhance the sucrose esters remaining with the fibers.

As shown, the data demonstrate a general inability to extract SEFOSE® out of the material after drying. On the other hand, when the fatty acids containing all saturated fatty acid chains are used instead of SEFOSE® (e.g., OLEAN®,

available from Procter & Gamble Chemicals (Cincinnati, Ohio)), nearly 100% of the material can be extracted using hot water (at or above 70° C.). OLEAN® is identical to SEFOSE® with the only change being saturated fatty acids attached (OLEAN®) instead of unsaturated fatty acids (SEFOSE®).

Another noteworthy aspect is that multiple fatty acid chains are reactive with the cellulose, and with the two saccharide molecules in the structure, the SEFOSE® gives rise to a stiff crosslinking network leading to strength improvements in fibrous webs such as paper, paperboard, air-laid and wet-laid non-wovens, and textiles.

Example 7. SEFOSE® Additions to Achieve Water Resistance

2 and 3 gram handsheets were made using both hardwood and softwood kraft pulps. When SEFOSE® was added to the 1% pulp slurry at a level of 0.1% or greater and water was drained forming the handsheet, SEFOSE® was retained with the fibers, where it imparted water resistance. From 0.1% to 0.4% SEFOSE®, water beaded on the surface for a few seconds or less. After SEFOSE® loading went above 0.4%, the time of water resistance quickly increased to minutes and then to hours for loading levels greater than 1.5%.

Example 8. Production of Bulky Fibrous Material

Addition of SEFOSE® to pulp acts to soften the fibers, increase space between them increasing bulk. For example, a 3% slurry of hardwood pulp containing 125 g (dry) of pulp was drained, dried and found to occupy 18.2 cubic centimeters volume. 12.5 g of SEFOSE® was added to the same 3% hardwood pulp slurry that contained an equivalent of 125 g dry fiber. Upon draining the water and drying, the resulting mat occupied 45.2 cubic centimeters.

30 g of a standard bleached hardwood kraft pulp (produced by Old Town Fuel and Fiber, LLC, Old Town, Me.) was sprayed with SEFOSE® that had been warmed to 60° C. This 4.3  $\text{cm}^3$  was placed in a disintegrator for 10,000 rpm and essentially repulped. The mixture was poured through a handsheet mold and dried at 105° C. The resulting hydrophobic pulp occupied a volume of 8.1  $\text{cm}^3$ . A 2 inch square of this material was cut and placed in a hydraulic press with 50 tons of pressure applied for 30 seconds. The volume of the square was reduced significantly but still occupied 50% more volume than the same 2 inch square cut for the control with no pressure applied.

It is significant that not only is an increase in bulk and softness observed, but that a forcibly repulped mat when the water was drained resulted in a fiber mat where all of the hydrophobicity was retained. This quality, in addition to the observations that water cannot be easily "pushed" past the low surface energy barrier into the sheet, is of value. Attachment of hydrophobic single-chains of fatty acids do not exhibit this property.

55 While not being bound by theory, this represent additional evidence that SEFOSE® is reacting with the cellulose and that the OH groups on the surface of the cellulose fibers are no longer available to participate in subsequent hydrogen bonding. Other hydrophobic materials interfere with initial hydrogen bonding, but upon repulping this effect is reversed and the OH groups on the cellulose are free to participate in hydrogen bonding upon redrying.

Example 9. Bag Paper Testing Data

The following table (Table 7) illustrates properties imparted by coating 5-7 g/m<sup>2</sup> with a SEFOSE® and poly-

vinyl alcohol (PvOH) mixture onto an unbleached kraft bag stock (control). Also included for reference are commercial bags.

TABLE 7

| Bag Paper Tests        |                    |                               |             |
|------------------------|--------------------|-------------------------------|-------------|
| Paper Type             | Caliper (0.001 in) | Tensile (lb/in <sup>2</sup> ) | Burst (psi) |
| Trial bag (control)    | 3.26               | 9.45                          | 52.1        |
| Trial bag with SEFOSE® | 3.32               | 15.21                         | 62.6        |
| Sub Sandwich bag       | 2.16               | 8.82                          | 25.2        |
| Home Depot leaf bag    | 5.3                | 17.88                         | 71.5        |

As may be seen in the Table, tensile and burst increase with the coating of the control base paper with SEFOSE® and PvOH.

Example 10. Wet/Dry Tensile Strength

3 gram handsheets were made from bleached pulp. The following compares wet and dry tensile strength at different levels of SEFOSE® addition. Note that with these handsheets SEFOSE® was not emulsified into any coating, it was simply mixed into the pulp and drained with no other chemistry added (see Table 8).

TABLE 8

| Wet/Dry Tensile Strength |                                    |                                    |
|--------------------------|------------------------------------|------------------------------------|
| SEFOSE® Loading          | Wet Strength (lb/in <sup>2</sup> ) | Dry Strength (lb/in <sup>2</sup> ) |
| 0%                       | 0.29                               | 9.69                               |
| 0.5%                     | 1.01                               | 10.54                              |
| 1%                       | 1.45                               | 11.13                              |
| 5%                       | 7.22                               | 15.02                              |

Note also, that the 5% addition for the wet strength is not far below the dry strength of the control.

Example 11. Use of Esters Containing Less Than 8 Saturated Fatty Acids

A number of experiments were carried out with sucrose esters produced having less than 8 fatty acids attached to the sucrose moiety. Samples of SP50, SP10, SP01 and F20W (from Sisterna, The Netherlands) which contain 50, 10, 1 and essentially 0% monoesters, respectively. While these commercially available products are made by reacting sucrose with saturated fatty acids, thus relegating them less useful for further crosslinking or similar chemistries, they have been useful in examining emulsification and water repelling properties.

For example, 10 g of SP01 was mixed with 10 g of glyoxal in a 10% cooked PvOH solution. The mixture was “cooked” at 200° F. for 5 mins and applied via drawdown to a porous base paper made from bleached hardwood kraft. The result was a crosslinked waxy coating on the surface of the paper that exhibited good hydrophobicity. Where a minimum of 3 g/m<sup>2</sup> was applied, the resulting contact angle was greater than 100°. Since the glyoxal is a well-known crystallizer used on compounds having OH groups, this method is a potential means to affix fairly unreactive sucrose esters to a surface by bonding leftover alcohol groups on the sucrose ring with an alcohol group made available in the substrate or other coating materials.

Example 12. HST Data and Moisture Uptake

To demonstrate that SEFOSE® alone provides the water proofing properties observed, porous Twins River (Matawaska, Me.) base paper was treated with various amounts of SEFOSE (and PvOH or Ethylex 2025 to emulsify, applied by drawdown) and assayed by Hercules Size Test. The results are shown in Table 9.

TABLE 9

| HST Data with SEFOSE®. |                                 |                                   |
|------------------------|---------------------------------|-----------------------------------|
| HST-seconds            | SEFOSE® pickup g/m <sup>2</sup> | Emulsifier g/m <sup>2</sup>       |
| <1                     | —                               | —                                 |
| 2.7                    | 0 g/m <sup>2</sup>              | 2.7 g/m <sup>2</sup> PvOH         |
| 16.8                   | 0 g/m <sup>2</sup>              | 4.5 g/m <sup>2</sup> Ethylex 2025 |
| 65                     | 2.2 g/m <sup>2</sup>            | 2.3 g/m <sup>2</sup> Ethylex 2025 |
| 389.7                  | 1.6 g/m <sup>2</sup>            | 1.6 g/m <sup>2</sup> PvOH         |
| 533                    | 3.0 g/m <sup>2</sup>            | 4.0 g/m <sup>2</sup> PvOH         |
| 1480                   | 5.0 g/m <sup>2</sup>            | 5.0 g/m <sup>2</sup> Ethylex 2025 |
| 2300+                  | 5.0 g/m <sup>2</sup>            | 5.0 g/m <sup>2</sup> PvOH         |

As can be seen in Table 9, increased SEFOSE® applied to the surface of the paper lead to increased water resistance (as shown by increased HST in seconds).

This may also be seen using coatings of a saturated sucrose ester product. For this particular example, the product, F20W (available from Sisterna, The Netherlands) is described as a very low % monoester with most molecules in the 4-8 substitution range. Note that the F20W product pickup is only 50% of the total coating, as it was emulsified with PvOH using equal parts of each to make a stable emulsion. So, where the pickup is labeled “0.5 g/m<sup>2</sup>” there is also the same pickup of PvOH giving a total pickup of 1.0 g/m<sup>2</sup>. Results are shown in Table 10.

TABLE 10

| HST Data F20W. |                      |
|----------------|----------------------|
| HST-Seconds    | Sisterna F20W pickup |
| <1             | 0                    |
| 2.0            | 0.5 g/m <sup>2</sup> |
| 17.8           | 1.7 g/m <sup>2</sup> |
| 175.3          | 2.2 g/m <sup>2</sup> |
| 438.8          | 3.5 g/m <sup>2</sup> |
| 2412           | 4.1 g/m <sup>2</sup> |

As can be seen from Table 10, again, increase F20W increases the water resistance of the porous sheet. Thus, the applied sucrose fatty acid ester itself is making the paper water resistance.

That the water resistance is not simply due to the presence of a fatty acid forming an ester bond with the cellulose, softwood handsheets (bleached softwood kraft) were loaded with SEFOSE® and oleic acid was directly added to the pulp, where the oleic acid forms an ester bond with the cellulose in the pulp. The mass at time zero represents the “bone dry” mass of the handsheets taken out of the oven at 105° C. The samples were placed in a controlled humidity room maintained at 50% RH. The change in mass is noted over time (in minutes). The results are shown in Tables 11 and 12.

TABLE 11

| Time<br>(Min) | Moisture Uptake SEFOSE ®. |                 |         |
|---------------|---------------------------|-----------------|---------|
|               | 2%<br>SEFOSE ®            | 30%<br>SEFOSE ® | Control |
| 0             | 3.859                     | 4.099           | 3.877   |
| 1             | 3.896                     | 4.128           | 3.911   |
| 3             | 3.912                     | 4.169           | 3.95    |
| 5             | 3.961                     | 4.195           | 3.978   |
| 10            | 4.01                      | 4.256           | 4.032   |
| 15            | 4.039                     | 4.276           | 4.054   |
| 30            | 4.06                      | 4.316           | 4.092   |
| 60            | 4.068                     | 4.334           | 4.102   |
| 180           | 4.069                     | 4.336           | 4.115   |

TABLE 12

| Time (hrs) | Moisture Uptake Oleic Acid. |                |         |
|------------|-----------------------------|----------------|---------|
|            | 30% Oleic Acid              | 50% Oleic Acid | Control |
| 0          | 4.018                       | 4.014          | 4.356   |
| 0.5        | 4.067                       | 4.052          | 4.48    |
| 2          | 4.117                       | 4.077          | 4.609   |
| 3          | 4.128                       | 4.08           | 4.631   |
| 5          | 4.136                       | 4.081          | 4.647   |
| 21         | 4.142                       | 4.083          | 4.661   |

Note the difference here where oleic acid is directly added to the pulp forming an ester bond greatly slows moisture uptake. In contrast, only 2% SEFOSE® slows moisture uptake, at higher concentrations, SEFOSE® does not. As such, while not being bound by theory, the structure of the SEFOSE® bound material cannot be simply explained by the structure formed by simple fatty acid esters and cellulose.

#### Example 13. Saturated SFAEs

The saturated class of esters are waxy solids at room temperature which, due to saturation, are less reactive with the sample matrix or itself. Using elevated temperatures (e.g., at least 40° C. and for all the ones tested above 65° C.) these material melt and may be applied as a liquid which then cools and solidifies forming a hydrophobic coating. Alternatively, these materials may be emulsified in solid form and applied as an aqueous coating to impart hydrophobic characteristics.

The data shown here represent HST (Hercules Size test) readings obtained from papers coated with varying quantities of saturated SFAEs.

A #45, bleached, hardwood kraft sheet obtained from Turner Falls paper was used for test coatings. The Gurley porosity measured approximately 300 seconds, representing a fairly tight base sheet. S-370 obtained from Mitsubishi Foods (Japan) was emulsified with Xanthan Gum (up to 1% of the mass of saturated SFAE formulation) before coating.

Coat weight of saturated SFAE formulation (pounds per ton) HST (average of 4 measurements per sample).

TABLE 13

| Coat<br>weight of S-370 (pounds per ton) | HST (average of 4 measurements per sample) |             |
|------------------------------------------|--------------------------------------------|-------------|
|                                          | Control only #0                            | 4 seconds   |
| Control only #0                          |                                            | 4 seconds   |
| #45                                      |                                            | 140 seconds |
| #65                                      |                                            | 385 seconds |

TABLE 13-continued

| Coat<br>weight of S-370 (pounds per ton) | HST (average of 4 measurements per sample) |              |
|------------------------------------------|--------------------------------------------|--------------|
|                                          | #100                                       | 839 seconds  |
| #150                                     |                                            | 1044 seconds |
| #200                                     |                                            | 1209 seconds |

Lab data generated also supports that limited amounts of saturated SFAE may enhance water resistance of coatings that are designed for other purposes/applications. For example, saturated SFAE was blended with Ethylex starch and polyvinyl alcohol based coatings and increased water resistance was observed in each case.

The examples below were coated on a #50, bleached recycled base with a Gurley porosity of 18 seconds.

100 grams of Ethylex 2025 were cooked at 10% solids (1 liter volume) and 10 grams of S-370 were added in hot and mixed using a Silverson homogenizer. The resulting coating was applied using a common benchtop drawdown device and the papers were dried under heat lamps.

At 300#/ton coat weight, the starch alone had an average HST of 480 seconds. With the same coat weight of the starch and saturated SFAE mixture, the HST increased to 710 seconds.

25 Enough polyvinyl alcohol (Selvol 205S) was dissolved in hot water to achieve a 10% solution. This solution was coated on the same #50 paper described above and had an average HST of 225 at 150 pounds/ton of coat weight. Using this same solution, S-370 was added to achieve a mixture in which contained 90% PVOH/10% S-370 on a dry basis (i.e., 90 ml water, 9 grams PvOH, 1 gram S-370): average HST increased to 380 seconds.

30 Saturated SFAEs are compatible with prolamines (specifically, zein; see U.S. Pat. No. 7,737,200, herein incorporated by reference in its entirety). Since one of the major barriers to commercial production of the subject matter of said patent is that the formulation be water soluble: the addition of saturated SFAEs assists in this manner.

#### Example 14. Other Saturated SFAEs

40 Size press evaluations of saturated SFAE based coatings were done on a bleached lightweight sheet (approx. 35 #) that had no sizing and relatively poor formation. All evaluations were done using Exceval HR 3010 PvOH cooked to emulsify the saturated SFAE. Enough saturated SFAE was added to account for 20% of the total solids. The focus was on evaluating the S-370 vs the C-1800 samples (available from Mitsubishi Foods, Japan). Both of these esters performed better than the control, some of the key data are shown in Table 14:

TABLE 14

|                             | Average HST | Kit Value |
|-----------------------------|-------------|-----------|
| 10% polyvinyl alcohol alone | 38 sec.     | 2         |
| PVOH with S-370             | 85 sec.     | 3         |
| PVOH with C-1800            | 82 sec.     | 5         |

60 Note that the saturated compounds appear to give an increase in kit, with both the S-370 and the C-1800 yielding a ~100% increase in HST.

#### Example 15. Wet Strength Additive

65 Laboratory testing has shown that the chemistry of the sucrose esters can be tuned to achieve a variety of properties,

including use as a wet strength additive. When the sucrose esters are made by attaching saturated groups to each alcohol functionality on the sucrose (or other polyol), the result is a hydrophobic, waxy substance having low miscibility/solubility in water. These compounds may be added to cellulosic materials to impart water resistance either internally or as a coating, however; since they are not chemically reacted to each other or any part of the sample matrix they are susceptible to removal by solvents, heat and pressure.

Where waterproofing and higher levels of water resistance are desired, sucrose esters containing unsaturated functional groups may be made and added to the cellulosic material with the goal of achieving oxidation and/or crosslinking which helps fix the sucrose ester in the matrix and render it highly resistant to removal by physical means. By tuning the number of unsaturated groups as well as the size of the sucrose esters, a means is obtained for crosslinking to impart strength, yet with a molecule that is not optimal for imparting water resistance.

The data shown here is taken by adding SEFOSE® to a bleached kraft sheet at varying levels and obtaining wet tensile data. The percentages shown in the table represent the percent sucrose ester of the treated 70 #bleached paper (see Table 15).

TABLE 15

| % SEFOSE ®    | Load  | Strain/Modulus |
|---------------|-------|----------------|
| 0%            | 4.98  | 0.93/89.04     |
| 1%            | 5.12  | 1.88/150.22    |
| 5%            | 8.70  | 0.99/345.93    |
| 10%           | 10.54 | 1.25/356.99    |
| Dry/untreated | 22.67 |                |

The data illustrate a trend in that adding unsaturated sucrose esters to papers increases the wet strength as loading level increases. The dry tensile shows the maximum strength of the sheet as a point of reference.

Example 16. Method of Producing Sucrose Esters Using Acid Chlorides

In addition to making hydrophobic sucrose esters via transesterification, similar hydrophobic properties can be achieved in fibrous articles by directly reacting acid chlorides with polyols containing analogous ring structures to sucrose.

For example, 200 grams of palmitoyl chloride (CAS 112-67-4) were mixed with 50 grams of sucrose and mixed at room temperature. After mixing the mixture was brought to 100° F. and maintained at that temperature overnight (ambient pressure). The resulting material was washed with acetone and deionized water to remove any unreacted or hydrophilic materials. Analysis of remaining material using C-13 NMR showed a significant quantity of hydrophobic sucrose ester had been made.

While it has been shown (by BT3 and others) that the addition of fatty acid chlorides to cellulosic materials could impart hydrophobic properties, the reaction itself is undesirable on site as the by-product given off, gaseous HCl, creates a number of problems including corrosion of surrounding materials and is hazardous to workers and surrounding environment. One additional problem created by the production of hydrochloric acid is that as more is formed, i.e., more polyol sites are reacted, the weaker the fibrous composition becomes. Palmitoyl chloride was

reacted in increasing amounts with cellulose and cotton materials and as hydrophobicity increased, strength of the article decreased.

The reaction above was repeated several times using 200 grams of R—CO-chloride reacted with 50 grams each of other similar polyols, including corn starch, xylan from birch, carboxymethylcellulose, glucose and extracted hemi-celluloses.

10

Example 17. Peel Test

Peel test utilizes a wheel between the two jaws of the tensile tester to measure force needed to peel tape off from a paper's surface as a reproducible angle (ASTM D1876; e.g., 100 Series Modular Peel Tester, TestResources, Shakopee, Minn.).

For this work, bleached kraft paper with high Gurley (600 seconds) from Turner Falls paper (Turner's Falls, Mass.) was used. This #50 pound sheet represents a fairly tight, but quite absorbent sheet.

When the #50 pound paper was coated with 15% Ethylex starch as a control, the average force (over 5 samples) that was needed was 0.55 pound/inch. When treated with the same coating but with SEFOSE® substituted for 25% of the Ethylex starch (so 25% pickup is SEFOSE®, 75% is still Ethylex) the average force decreased to 0.081 pounds/inch. With a 50% substitution of SEFOSE® for the Ethylex, the force needed decreased to less than 0.03 pounds per inch.

The preparation of this paper is in accord with TAPPI standard method 404 for determining tensile strength of papers.

Finally, the same paper was used with S-370 at a loading rate of 750 pounds per ton—which effectively fills all the pores in the sheet creating a complete physical barrier. This indeed passes a TAPPI kit 12 on the flat. This brief experiment shows that it is possible to get grease resistance using saturated SFAE varieties.

35

Example 18. SFAE Blends

Materials

SFAEs were obtained from Fooding Group Ltd (SE-15, HLB=15; Shanghai, CHINA) and Mitsubishi Chemical Foods Corporation (C-1803, HLB=3; Tokyo, JAPAN). Esters were blended at a 50:50 ratio and heated in water. Blend A comprises SE-15 and C-1803. Blend B comprises SE-15, C-1803 and BARRISURF LX dry clay (Imerys, S. A., Paris, FRANCE).

A 40 #unbleached, unsized paper was coated with the aqueous ester blend with a coat weight of 7 g/m<sup>2</sup>. Control papers were left untreated but dried under the same conditions. After drying at 100° C. in an oven for 5 minutes, data was observed as shown in Table 16.

TABLE 16

|         | 3M | WCA | OCA | HST |
|---------|----|-----|-----|-----|
| Control | 0  | <60 | 0   | <2  |
| A       | 5  | 98  | 71  | 250 |
| B       | 6  | 98  | 71  | 280 |

3M = 3M kit;

WCA = water contact angle;

OCA = oil contact angle;

HST = Hercules size test.

60

65

The addition of 10% by weight of dry clay to the aqueous ester dispersion and applied to the same papers at the same coat weight improved HST and the 3M kit (see Table 16).

It seems evident that the blends alone are all that is necessary to achieve water and grease resistance. While not being bound by theory, it is noteworthy here that the ester blends may allow new ways of formulating for those who need mid-range kit and have no coater capability on site. Additionally, it may allow for the achievement of higher kit with some levels of pigment added, which might be of interest especially to talc suppliers who have experimented in the OGR markets already.

The following is an example of how blending unsaturated esters can improve properties.

SFAEs were obtained from Fooding Group Ltd (SE-15, HLB=15; SE-30, HLB=7; Shanghai, CHINA) and Mitsubishi Chemical Foods Corporation (S-370, HLB=3; Tokyo, JAPAN). Esters were blended in equal parts and heated in water. The coatings were made to 10% solids and applied to an unbleached bag stock paper. Coat weight was approximately 7 g/m<sup>2</sup> as applied by hand drawdown.

| Composition             | HST | Contact angle |
|-------------------------|-----|---------------|
| Base paper - no coating | 0   | 0             |
| SE-30                   | 22  | 75            |
| SE-15                   | 122 | 60            |
| S-370                   | 8   | 110           |
| S-370/SE 15/SE-30       | 110 | 95            |

This data shows that by blending esters, most of the HST of the SE-15 and most of the contact angle of the S-370 is maintained by using the above blend. Note that the HST of three blended SFAEs is reduced by only 10-20% even though the SE-15 component has been reduced by 66%.

#### Other Uses

Cup base stock was found to be heavily treated with rosin to increase water resistance. However, the Gurley on this board was found to be 50 seconds indicating a fairly porous board. This material is repulsive and steam quickly penetrates to soften it. Pure SEFOSE® was applied to this board and dried in an oven at 100° C. overnight. The resulting material had a plastic like feel and was completely waterproof. By mass, it was 50% (wt/wt) cellulose/50% (wt/wt) SEFOSE®. The Gurley was too high to measure. Submerging a sample in water for 7 days did not significantly soften the material, however, from greenhouse data it seems to biodegrade in approximately 150 days. Common tapes and glues would not stick to this composite material.

Experiments with saturated SFAE and zein have been carried out, as zein has been shown to impart grease resistance to paper. Stable aqueous dispersions of zein (up to 25% in water) to which saturated SFAE was added from 2 to 5% were generated. Observations demonstrated that saturated SFAE "locks down" zein on paper by imparting water resistance (in addition to grease resistance) to the formulation.

Although the invention has been described with reference to the above examples, it will be understood that modifications and variations are encompassed within the spirit and scope of the invention. Accordingly, the invention is limited only by the following claims. All references disclosed herein are hereby incorporated by reference in their entireties.

#### What is claimed:

1. A barrier coating, comprising:  
at least two polyol fatty acid esters (PFAE) or saccharide fatty acid esters (SFAE),

wherein at least one of the at least two PFAEs or SFAEs has an HLB value of equal to or less than 3 and at least one of the at least two PFAEs or SFAEs has an HLB value of equal to or greater than 7, and

5 wherein at least one PFAE or SFAE is a penta-, hexa-, hepta, or octa-ester or a mixture thereof.

2. The barrier coating of claim 1, wherein each one of the PFAEs or SFAEs possesses a different degree of substitution (DS).

10 3. The barrier coating of claim 1, wherein when said coating consists essentially of a first PFAE or SFAE having an HLB value of 3 and second PFAE or SFAE having an HLB value of greater than 7, and a Hercules Size Test (HST) value of a substrate comprising the coating is greater than the combined HST values of a coating containing only the first or second PFAEs or SFAEs.

15 4. The barrier coating of claim 2, wherein said at least two PFAEs or SFAEs are present in the barrier coating at a sufficient concentration to cause a surface of an article containing the coating to become substantially resistant to application of water, oil and/or grease in the absence of a secondary lipophobe or hydrophobe.

5. The barrier coating of claim 1, wherein one of the at least two SFAEs contains 1 to 5 fatty acid moieties.

25 6. The barrier coating of claim 1, wherein the fatty acid moieties are saturated or are a combination of saturated and unsaturated fatty acids.

30 7. The barrier coating of claim 1, further comprising one or more compositions including clay, precipitated calcium carbonate (PCC), ground calcium carbonate (GCC), natural and/or synthetic latexes, prolamines, polyvinyl alcohol (PvOH), TiO<sub>2</sub>, talc, glyoxal, modified starches, kaolin and combinations thereof, and optionally, one or more additives selected from the group consisting of starches, modified starches, hydrocarbon resins, polymers, waxes, polysaccharides, proteins, dyestuffs, optical brightening agents, and combinations thereof.

35 8. The barrier coating of claim 1, wherein the coating comprises clay, GCC or PCC.

40 9. The barrier coating of claim 8, wherein at least one of the at least two PFAEs or SFAEs is a monoester or a diester.

10. The barrier coating of claim 1, wherein the barrier coating is biodegradable and/or compostable.

45 11. An article, comprising:  
a substrate; and  
the barrier coating of claim 1 adhered to a surface of the substrate,

wherein the substrate is selected from the group consisting of paper, paperboard, paper pulp, a carton for food storage, fruit, a bag for food storage, a shipping bag, a container for coffee or tea, a tea bag, bacon board, diapers, weed-block/barrier fabric or film, mulching film, plant pots, packing beads, bubble wrap, oil absorbent material, laminates, envelopes, gift cards, credit cards, gloves, raincoats, OGR paper, a shopping bag, a compost bag, release paper, eating utensil, container for holding hot or cold beverages, cup, paper towels, plate, a bottle for carbonated liquid storage, insulating material, a bottle for non-carbonated liquid storage, film for wrapping food, a garbage disposal container, a food handling implement, a lid for a cup, a fabric fibre, a water storage and conveying implement, a storage and conveying implement for alcoholic or non-alcoholic drinks, an outer casing or screen for electronic goods, an internal or external piece of furniture, a curtain, upholstery, film, box, sheet, tray, pipe, water conduit, packaging for pharmaceutical products, clothing, medi-

37

- cal device, contraceptive, camping equipment, cellulosic material that is molded and combinations thereof.
12. The article according to claim 11, wherein a surface of the article having the barrier coating has a water contact angle of equal to or greater than 90°.

13. The article according to claim 11, wherein a surface of the article having the barrier coating has a TAPPIT 559 KIT test value of at least 5.

14. The article according to claim 11, wherein a surface of the article having the barrier coating has a TAPPIT 559 KIT test value of at least 7 and a water contact angle of equal to or greater than 90°.

15. A method for tuneably derivatizing a cellulose-based material for lipid and water resistance, the method comprising:

10 contacting a cellulose-based material with the barrier coating of claim 1; and  
 exposing the contacted cellulose-based material to heat, radiation, a catalyst or combination thereof for a sufficient time to adhere the barrier coating to the cellulose based material.

15 16. The method of claim 15, wherein the cellulose-based material having the barrier coating adhered thereto is sub-

38

stantially resistant to application of water, oil and/or grease in the absence of a secondary lipophobe or hydrophobe.

17. The method of claim 15, wherein the cellulose-based material having the barrier coating adhered thereto is substantially resistant to application of water and grease.

18. A barrier coating, comprising:  
 at least two polyol fatty acid esters (PFAEs) or saccharide fatty acid esters (SFAEs); and  
 one or more inorganic particles,

5 wherein at least one of the at least two PFAEs or SFAEs has an HLB value of equal to or less than 3 and at least one of the at least two PFAEs or SFAEs has an HLB value of equal to or greater than 7, and  
 wherein at least one PFAE or SFAE is a penta-, hexa-, hepta, or octa-ester or a mixture thereof.

19. The barrier coating of claim 18, wherein the inorganic particles are selected from the group consisting of clay, talc, precipitated calcium carbonate, ground calcium carbonate, TiO<sub>2</sub> and combinations thereof.

20 20. The barrier coating of claim 18, wherein each one of the PFAEs or SFAEs possesses a different degree of substitution (DS).

\* \* \* \* \*